



US006479222B1

(12) **United States Patent**  
Jones et al.

(10) **Patent No.:** US 6,479,222 B1  
(45) **Date of Patent:** \*Nov. 12, 2002

(54) **PROTECTIVE OVERCOAT FOR  
PHOTOGRAPHIC ELEMENTS**

(75) Inventors: **Tamara K. Jones**, Rochester; **Lloyd A. Lobo**, Webster; **Mridula Nair**, Penfield; **Kevin M. O'connor**, Webster; **Tiecheng A. Qiao**, Webster; **Yongcai Wang**, Webster; **Thomas H. Whitesides**; **Hwei-Ling Yau**, both of Rochester, all of NY (US)

(73) Assignee: **Eastman Kodak Company**, Rochester, NY (US)

(\*) Notice: Subject to any disclaimer, the term of this patent is extended or adjusted under 35 U.S.C. 154(b) by 0 days.

This patent is subject to a terminal disclaimer.

(21) Appl. No.: **09/621,267**

(22) Filed: **Jul. 21, 2000**

(51) **Int. Cl.**<sup>7</sup> ..... **G03C 1/76**; G03C 11/06; G03C 11/08

(52) **U.S. Cl.** ..... **430/350**; 430/523; 430/531; 430/536; 430/537; 430/961; 430/533

(58) **Field of Search** ..... 430/350, 523, 430/531, 533, 536, 537, 961

(56) **References Cited**

U.S. PATENT DOCUMENTS

2,706,686 A 4/1955 Hilborn

|              |   |         |                   |       |         |
|--------------|---|---------|-------------------|-------|---------|
| 4,554,235 A  | * | 11/1985 | Adair et al.      | ..... | 430/961 |
| 4,797,353 A  |   | 1/1989  | Yamada et al.     | ..... | 430/434 |
| 5,177,128 A  |   | 1/1993  | Lindemann et al.  | ..... | 524/44  |
| 5,695,920 A  |   | 12/1997 | Anderson et al.   | ..... | 430/531 |
| 5,804,360 A  |   | 9/1998  | Schell et al.     | ..... | 430/535 |
| 5,846,699 A  |   | 12/1998 | Wang et al.       | ..... | 430/536 |
| 5,853,926 A  |   | 12/1998 | Bohan et al.      | ..... | 430/350 |
| 5,856,051 A  |   | 1/1999  | Yau et al.        | ..... | 430/350 |
| 5,910,401 A  |   | 6/1999  | Anderson et al.   | ..... | 430/531 |
| 6,077,648 A  | * | 6/2000  | Nair et al.       | ..... | 430/531 |
| 6,153,363 A  | * | 11/2000 | Nair et al.       | ..... | 430/531 |
| 6,187,517 B1 | * | 2/2001  | Whitesides et al. | ..... | 430/961 |
| 6,190,843 B1 | * | 2/2001  | Yau et al.        | ..... | 430/961 |
| 6,194,130 B1 | * | 2/2001  | Nair et al.       | ..... | 430/531 |
| 6,274,298 B1 | * | 8/2001  | Nair et al.       | ..... | 430/533 |

OTHER PUBLICATIONS

Japanese Patent Abstract 6067328 Mar. 1994.

\* cited by examiner

*Primary Examiner*—Richard L. Schilling

(74) *Attorney, Agent, or Firm*—Chris P. Konkol

(57) **ABSTRACT**

The present invention is a photographic element which includes a support, at least one silver halide emulsion layer superposed on the support and a processing-solution-permeable protective overcoat overlying the silver halide emulsion layer that becomes water-resistant in the final product without lamination or fusing. The present invention is also directed to a method of making a photographic print involving developing the photographic element.

**15 Claims, No Drawings**

## PROTECTIVE OVERCOAT FOR PHOTOGRAPHIC ELEMENTS

### FIELD OF THE INVENTION

The present invention relates to photographic imaging elements having a protective overcoat that resists fingerprints, common stains, and spills. More particularly, the present invention provides a processing-solution-permeable overcoat that becomes water resistant in the photochemically processed product. The overcoat formulation comprises at least one water-dispersible hydrophobic polymer interspersed with a water-soluble polymer. During development or thereafter, before drying, the water-soluble polymer is removed to a significant extent, facilitating coalescence of the residual water-dispersible polymer, thereby forming a water-resistant continuous protective overcoat.

### BACKGROUND OF THE INVENTION

Silver halide photographic elements contain light sensitive silver halide in a hydrophilic emulsion. An image is formed in the element by exposing the silver halide to light, or to other actinic radiation, and developing the exposed silver halide to reduce it to elemental silver.

In color photographic elements, a dye image is formed as a consequence of silver halide development by one of several different processes. The most common is to allow a by-product of silver halide development, oxidized silver halide developing agent, to react with a dye forming compound called a coupler. The silver and unreacted silver halide are then removed from the photographic element, leaving a dye image.

In either case, formation of the image commonly involves liquid processing with aqueous solutions that must penetrate the surface of the element to come into contact with silver halide and coupler. Thus, gelatin or similar natural or synthetic hydrophilic polymers have proven to be the binders of choice for silver halide photographic elements. Unfortunately, when gelatin or similar polymers are formulated so as to facilitate contact between the silver halide crystals and aqueous processing solutions, the resultant coatings are not as fingerprint and stain resistant as would be desirable, particularly in view of the handling or environment that an imaged photographic element may commonly experience at various times and circumstances. Thus, fingerprints can permanently mark the imaged element. The imaged element can be easily stained by common household products, such as foods or beverages, for example, coffee spills.

There have been attempts over the years to provide protective layers for gelatin based photographic systems that will protect the images from damages by water or aqueous solutions. U.S. Pat. No. 2,173,480 describes a method of applying a colloidal suspension to moist film as the last step of photographic processing before drying. A series of patents describes methods of solvent coating a protective layer on the image after photographic processing is completed and are described in U.S. Pat. Nos. 2,259,009, 2,331,746, 2,798, 004, 3,113,867, 3,190,197, 3,415,670 and 3,733,293. U.S. Pat. No. 5,376,434 describes a protective layer formed on a photographic print by coating and drying a latex on a gelatin-containing layer bearing an image. The latex is a resin having a glass transition temperature of from 30° C. to 70° C. The application of UV-polymerizable monomers and oligomers on processed image followed by radiation expo-

sure to form crosslinked protective layer is described in U.S. Pat. Nos. 4,092,173, 4,171,979, 4,333,998 and 4,426,431. A drawback for both the solvent coating method and for the radiation cure method is the health and environmental concern of those chemicals or radiation to the coating operator. Another drawback is that the photographic materials need to be coated after the processing step. Thus, the processing equipment needs to be modified and the personnel running the processing operation need to be trained to apply the protective coating.

Various lamination techniques are known and practiced in the trade. U.S. Pat. Nos. 3,397,980, 3,697,277 and 4,999,266 describe methods of laminating a polymeric sheet film, as a protective layer, on a processed image. U.S. Pat. No. 5,447, 832 describes the use of a protective layer containing a mixture of high and low Tg latices as a water-resistant layer to preserve the antistat property of a  $V_2O_5$  layer through photographic processing. This protective layer is not applicable to the image formation layers, however, since it will detrimentally inhibit the photographic processing. U.S. Pat. No. 3,443,946 provides a roughened (matte) scratch-protective layer, but not one designed to be water-impermeable or resistant. U.S. Pat. No. 3,502,501 is intended to provide protection against mechanical damage only; the layer in question contains a majority of hydrophilic polymeric materials, and must be permeable to water in order to maintain processibility. U.S. Pat. No. 5,179,147 likewise provides an overcoat that is not water-protective.

Protective coatings that need to be applied to the image after it is formed, several of which were mentioned above, adds a significant cost to the final imaged product. A number of patents have been directed to water-resistant protective coatings that can be applied to a photographic element prior to development. For example, U.S. Pat. No. 2,706,686 describes the formation of a lacquer finish for photographic emulsions, with the aim of providing water-and fingerprint-resistance by coating the light-sensitive layer, prior to exposure, with a porous layer that has a high degree of water permeability to the processing solutions. After processing, the lacquer layer is fused and coalesced into a continuous, impervious coating. The porous layer is achieved by coating a mixture of a lacquer and a solid removable extender (ammonium carbonate), and removing the extender by sublimation or dissolution during processing. The overcoat as described is coated as a suspension in an organic solvent, and thus is not desirable for large-scale application. More recently, U.S. Pat. No. 5,853,926 to Bohan et al. discloses a protective coating for a photographic element, involving the application of an aqueous coating comprising polymer particles and a soft polymer latex binder. This coating allows for appropriate diffusion of photographic processing solutions, and does not require a coating operation after exposure and processing. Again, however, the hydrophobic polymer particles must be fused to form a protective coating that is continuous and water-impermeable.

U.S. Pat. No. 5,856,051 describes the use of hydrophobic particles with gelatin as the binder in an overcoat formulation. This invention demonstrated an aqueous coatable, water-resistant protective overcoat that can be incorporated into the photographic product, allows for appropriate diffusion of photographic processing solutions, and does not require a coating operation after exposure and processing. The hydrophobic polymers exemplified in U.S. Pat. No. 5,856,051 include polyethylene have a melting temperature (Tm) of 55 to 200° C., and are therefore capable of forming a water-resistant layer by fusing the layer at a temperature higher than the Tm of the polymer after the sample has been

processed to generate the image. The coating solution is aqueous and can be incorporated in the manufacturing coating operation without any equipment modification. Again, however, fusing is required by the photofinishing laboratories to render the protective overcoat water-resistant. Similarly, commonly assigned U.S. Ser. Nos. 09/353,939 and 09/548,514, respectively, describe the use of a polystyrene-based material and a polyurethane-based material, with gelatin as the binder, in an overcoat for a photographic element, which overcoat can be fused into a water resistant overcoat after photographic processing is accomplished to generate an image.

Commonly assigned U.S. Ser. No. 09/235,436 discloses the use of a processing solution permeable overcoat that is composed of a urethane-vinyl copolymer having acid functionalities. Commonly assigned U.S. Ser. Nos. 09/235,437 and 09/448,213 disclose the use of a second polymer such as a gelatin or polyvinyl alcohol to improve processibility and reduce coating defects.

It would be desirable provide an improved protective overcoat that is economical. It would be desirable to obtain a water-resistant protective overcoat for an photographically imaged element without the addition of laminating or fusing steps, without the need for high temperatures, and without requiring additional equipment to carry out photoprocessing.

#### SUMMARY OF THE INVENTION

The present invention is directed to a processing-solution-permeable overcoat for a photographic element that provides water resistance in the final product. For example, such a photographic element may comprise a support, at least one silver-halide emulsion layer superposed on the support, and overlying the silver-halide emulsion layer, a processing-solution-permeable protective overcoat composition that can be incorporated into or coated on the imaging element during manufacturing and that does not inhibit photographic processing. A component of the invention are hydrophobic polymer particles that are water-dispersible. The material of the invention can be introduced to the overcoat coating melt in a latex form or as a conventional colloidal dispersion in a hydrophilic binder. The presence of a hydrophilic component that is substantially washed out during processing allows photographic processing to proceed at an acceptable rate. The washing out of the hydrophilic component facilitates the coalescence of the hydrophobic materials in the final product, further facilitated by elevated temperatures commonly associated with drying.

In one embodiment of the invention, the overcoat composition applied to the imaging element comprises 30 to 95 weight percent, based on the dry laydown of the overcoat, of water-dispersible polymer particles having an average of between 0.01 to 0.5 micrometers, said water-dispersible polymer being characterized by a  $T_g$  (glass transition temperature) of between -40 and 80° C.

Another aspect of the invention provides for a method of forming an image in the imaging element described above and converting the overcoat into a water-resistant coating.

In another embodiment of the invention, a photographic element comprises: (a) a support; (b) at least one silver-halide emulsion layer superposed on a side of said support; and overlying the silver emulsion layer, (c) a processing-solution-permeable protective overcoat having a laydown of at least 0.54 g/m<sup>2</sup> (50 mg/ft<sup>2</sup>) made from an overcoat formulation that is substantially gelatin-free, comprising less than 5% crosslinked gelatin by weight of solids. In general, the overcoat composition preferably contains a water-

soluble, hydrophilic polymer that is typically noncrosslinked to facilitate its washing out during processing and, at least to some extent, to facilitate the coalescence of the water-dispersible polymer particles.

In another embodiment of the invention, the applied overcoat composition comprises about of 30 to 95% by weight of solids of water-dispersible polymer particle having an average particle size of less than 500 nm and a  $T_g$  between -40° C. and 80° C., and 5 to 70% by weight of solids of water-soluble hydrophilic polymer such that more than 30 weight percent of the water-soluble polymer is washed out during photographic processing; wherein the weight ratio of the hydrophobic polymer to the non-crosslinked hydrophilic polymer is between 60:40 to 85:15 and whereby the overcoat forms a water-resistant overcoat after photoprocessing without fusing.

#### DESCRIPTION OF THE PREFERRED EMBODIMENTS

The present invention provides a simple and inexpensive way to improve the water, stain and abrasion resistance of processed photographic elements. In accordance with the invention, the protective overcoat is applied over the photographic element prior to exposure and processing. In particular, a overcoat formulation according to the present invention is applied to the emulsion side of photographic products, particularly photographic prints, which may encounter frequent handling and abuse by end users.

By the term "water-resistant" is meant herein after ordinary photoprocessing and drying does not imbibe water or prevents or minimizes water-based stains from discoloring the imaged side of the photographic element. By the term "non-crosslinked gelatin" is meant gelatin that is water soluble.

By the term "elevated temperature", as used in this application, to dry and/or facilitate coalescence of the water-dispersible polymer, is herein meant a temperature of from 30 to 80° C., preferably 45 to 60° C. In contrast, fusing typically requires a pressure roller or belt and drying of the imaged element before fusing. Fusing generally requires higher temperatures, typically above the boiling point of water, usually above 100° C.

The present invention provides an improved overcoat formulation for the imaging side of an imaging element or material, including photographic prints, which encounter frequent handling and abuse by end users. The preferred overcoat formulation of this invention comprises 30 to 95% by weight (based on the dry laydown of the overcoat) of water-dispersible polymer particles of 0.01 to 0.5 micrometers in average size and 5 to 70% by weight of a hydrophilic polymer which is substantially uncrosslinked (based on the dry laydown of the overcoat).

In one embodiment, a water-resistant layer is facilitated by coalescing the residual water-dispersible polymer material in the imaging element at a temperature sufficiently high, preferably during the drying step, after the photographic material has been photochemically processed. The use of less than 5% by weight of crosslinked gelatin or other crosslinked hydrophilic polymer in the overcoat (as applied) is sufficient to allow proper coalescence of during such a drying step. It is noted that some gelatin from underlying layers in the photographic element may migrate into the overcoat, during manufacture or photochemical processing, for example, but any such migration is limited and, by definition, is not included in the composition formulation or in the applied overcoat. In one embodiment, less than 5%,

more preferably less than 3%, by weight of solids, of gelatin is included in the overcoat composition. Most preferably, essentially no gelatin is included in the overcoat formulation. In one embodiment, however, crosslinkable gelatin is applied over the emulsion layer, which becomes crosslinked during manufacture of the photographic element, but becomes digested and converted to substantially non-crosslinked gelatin in the final product, in which at least 95% of the gelatin is water soluble.

As indicated above, a photographic element according to the present invention comprises: (a) a support; (b) at least one silver-halide emulsion layer superposed on a side of said support; and (c) overlying the silver emulsion layer, a processing-solution-permeable protective overcoat having a laydown of at least 0.54 g/m<sup>2</sup> (50 mg/ft<sup>2</sup>) made from a formulation comprising less than 5%, by weight of solids, of crosslinked gelatin and further comprising 30 to 95% by weight of solids, preferably 60 to 90 weight percent, of water-dispersible polymer particles having an average particle size of less than 500 nm and a  $T_g$  between -40 to 80° C., preferably 10° C. to 60° C., and 5 to 70%, by weight of solids, preferably 10 to 40 weight percent, of a water-soluble hydrophilic polymer such that more than 30 weight percent of the water-soluble polymer is washed out during photographic processing; wherein the weight ratio of the water-dispersible polymer to the non-crosslinked hydrophilic polymer is between 50:50 to 90:10, preferably 60:40 to 85:15, whereby the overcoat forms a water-resistant overcoat after photoprocessing without fusing, namely by maintaining the photographic element at temperature less than 100° C.

The dispersions of hydrophobic polymers used in this invention are latexes or hydrophobic polymers of any composition that can be stabilized in an water-based medium. Such hydrophobic polymers are generally classified as either condensation polymer or addition polymers. Condensation polymers include, for example, polyesters, polyamides, polyurethanes, polyureas, polyethers, polycarbonates, poly-acid anhydrides, and polymers comprising combinations of the above-mentioned types. Addition polymers are polymers formed from polymerization of vinyl-type monomers including, for example, allyl compounds, vinyl ethers, vinyl heterocyclic compounds, styrenes, olefins and halogenated olefins, unsaturated acids and esters derived from them, unsaturated nitriles, vinyl alcohols, acrylamides and methacrylamides, vinyl ketones, multifunctional monomers, or copolymers formed from various combinations of these monomers. Such latex polymers can be prepared in aqueous media using well-known free radical emulsion polymerization methods and may consist of homopolymers made from one type of the above-mentioned monomers or copolymers made from more than one type of the above-mentioned monomers. Polymers comprising monomers which form water-insoluble homopolymers are preferred, as are copolymers of such monomers. Preferred polymers may also comprise monomers which give water-soluble homopolymers, if the overall polymer composition is sufficiently water-insoluble to form a latex. Further listings of suitable monomers for addition type polymers are found in U.S. Pat. No. 5,594,047 incorporated herein by reference. The polymer can be prepared by emulsion polymerization, solution polymerization, suspension polymerization, dispersion polymerization, ionic polymerization (cationic, anionic), Atomic Transfer Radical Polymerization, and other polymerization methods known in the art of polymerization. The selection of water-dispersible particles to be used in the overcoat is based on the material properties one wishes to have as the protective overcoat in addition to water resistance.

The water-dispersible polymer is selected so that fusing is not required, a potentially significant advantage compared to the prior art, for example U.S. Pat. No. 5,856,051, mentioned above. It has been found that once the hydrophilic polymer is removed (which may optionally involve being first hydrolyzed and degraded by proteolytic enzyme) and removed during photographic processing (including optional additional washing), the selected water-dispersible particles will coalesce without fusing (which they would not do in the presence of substantial amounts of crosslinked gelatin or the like).

In a preferred embodiment of the invention, the water-dispersible polymer is a substantially amorphous, thermoplastic polymer having ionized or ionizable groups or moieties in sufficient number to provide water dispersibility prior to coating. In addition to water-resistance, the polymer dispersions in the finally processed product preferably provides further advantageous properties such as good chemical and stain resistance, wet-abrasion resistance, fingerprint resistance, toughness, elasticity, durability, and/or resistance to various oils.

In the case of carboxylic acid ionic groups, the polymer can be characterized by the acid number, which is preferably greater than or equal to 5 and relatively permeable to water at a pH of greater than 7. Preferably, the acid number is less than or equal to 40, more preferably less than or equal to 30. Preferably, the pH of the developing solution is greater than 8, preferably greater than 9. The water-reducible water-dispersible polymer particles comprising ionized or ionizable groups may be branched, unbranched, crosslinked, uncrosslinked.

In accordance with this invention, the protective overcoat preferably comprises, in addition to the water-dispersible polymer described above, at least one water-soluble hydrophilic polymer. Examples of such water-soluble polymers that may be added include polyvinyl alcohol, cellulose ethers, poly(N-vinyl amides), polyacrylamides, polyesters, poly(ethylene oxide), dextrans, starch, uncrosslinked gelatin, whey, albumin, poly(acrylic acid), poly(ethyl oxazolines), alginates, gums, poly(methacrylic acid), poly(oxymethylene), poly(ethyleneimine), poly(ethylene glycol methacrylate), poly(hydroxy-ethyl methacrylate), poly(vinyl methyl ether), poly(styrene sulfonic acid), poly(ethylene sulfonic acid), poly(vinyl phosphoric acid) and poly(maleic acid) and the like. Such materials are included in "Handbook of Water-Soluble Gums and Resins" by Robert I. Davidson (McGraw-Hill Book Company, 1980) or "Organic Colloids" by Bruno Jurgensons (Elsevier Publishing Company, 1958). In a preferred embodiment, the polymer is polyvinyl alcohol, which polymer has been found to yield coatings that are relatively uniform and to enhance the diffusion rate of the developer into the underlying emulsions.

The preferred hydrophilic polymer is polyvinyl alcohol. The term "polyvinyl alcohol" referred to herein means a polymer having a monomer unit of vinyl alcohol as a main component. Polyvinyl alcohol is typically prepared by substantial hydrolysis of polyvinyl acetate. Such a "polyvinyl alcohol" includes, for example, a polymer obtained by hydrolyzing (saponifying) the acetate ester portion of a vinyl acetate polymer (exactly, a polymer in which a copolymer of vinyl alcohol and vinyl acetate is formed), and polymers obtained by saponifying a trifluorovinylacetate polymer, a vinyl formate polymer, a vinyl pivalate polymer, a tert-butylvinylether polymer, a trimethylsilylvinylether polymer, and the like (the details of "polyvinyl alcohol" can be referred to, for example, "World of PVA", Edited by the

Poval Society and Published by Kobunshi Kankoukai, Japan, 1992 and "Poval", Edited by Nagano et al. and Published by Kobunshi Kankoukai, Japan, 1981). The degree of hydrolysis (or saponification) in the polyvinyl alcohol is preferably at least about 70% or more, more preferably at least about 80%. Percent hydrolysis refers to mole percent. For example, a degree of hydrolysis of 90% refers to polymers in which 90 mol % of all copolymerized monomer units of the polymer are vinyl alcohol units. The remainder of all monomer units consists of monomer units such as ethylene, vinyl acetate, vinyl trifluoroacetate and other comonomer units which are known for such copolymers. Most preferably, the polyvinyl alcohol has a weight average molecular weight (MW) of less than 150,000, preferably less than 100,000, and a degree of hydrolysis greater than 70%. If the MW is greater than 100,000, the degree of hydrolysis is preferably less than 95%. Preferably, the degree of hydrolysis is 85 to 90% for a polyvinyl alcohol having a weight average MW of 25,000 to 75,000. These preferred limitations may provide improved manufacturability and processibility. The polyvinyl alcohol is selected to make the coating wettable, readily processable, and in a

amounts are not used as this will decrease the permeability of the processing solution. The crosslinker may be added to the mixture of water-dispersible component and any additional polymers.

The optimal amount of the water-soluble polymer may depend on the amount of dry coverage of water-dispersible polymer. For example, in the case of the combination of a polyurethane polymer and a polyvinyl alcohol polymer, if coverage of a polyurethane polymer is 1.08 g/m<sup>2</sup> (100 mg/ft<sup>2</sup>) or less, then about 20% or less of polyvinyl alcohol, by weight of the polyurethane, provides good results, whereas for higher coverage, for example (1.88 g/m<sup>2</sup>) 175 mg/ft<sup>2</sup>, greater than about 25% of the polyvinyl alcohol provides comparably good results. In one preferred embodiment, the water-dispersible polymer of this invention are polyurethanes, preferably segmented polyurethanes. Polyurethanes are the polymerization reaction product of a mixture comprising polyol monomers and polyisocyanate monomers. A preferred segmented polyurethane is described schematically by the following structure (I):



35

substantial amount, to readily, not sluggishly, come out of the coating during processing, thereby yielding the final water-resistant product. The optimal amount of polyvinyl alcohol depends on the amount of dry coverage of water-dispersible polymer. In one preferred embodiment of the invention, the polyvinyl alcohol is present in the overcoat in the amount between 1 and 60 weight percent of the water-dispersible polymer, preferably between 5 and 50 weight percent of the water-dispersible polymer, most preferably between 10 and 45 weight percent of the water-dispersible polymer.

Without wishing to be bound by theory, it is believed that the water-soluble polymer and water-dispersible polymer form a biphasic mixture, which allows the formation of a water-resistant overcoat that does not require fusing, merely elevated temperatures preferably up to about 60° C. It is believed that fusing is not required for several reasons: (a) the substantial absence of cross-linked gelatin and other such crosslinked polymers, and (b) the selection of a water-dispersible polymer that is believed to form a biphasic system with the hydrophilic water-soluble polymer, but which after processing forms a water-resistant overcoat.

Optionally, the coating composition in accordance with the invention may also contain suitable crosslinking agents for crosslinking the water-dispersible polymer. Such an additive can improve the adhesion of the overcoat layer to the substrate below as well as contribute to the cohesive strength of the layer. Crosslinkers such as epoxy compounds, polyfunctional aziridines, methoxyalkyl melamines, triazines, polyisocyanates, carbodiimides, polyvalent metal cations, and the like may all be considered. If a crosslinker is added, care must be taken that excessive



Structure I

wherein R<sub>1</sub> is preferably a hydrocarbon group having a valence of two, more preferably containing a substituted or unsubstituted, cyclic or non-cyclic, aliphatic or aromatic group, most preferably represented by one or more of the following structures:



and wherein A represents a polyol, such as a) a dihydroxy polyester obtained by esterification of a dicarboxylic acid such as succinic acid, adipic acid, suberic acid, azelaic acid, sebatic acid, phthalic, isophthalic, terephthalic, tetrahydrophthalic acid, and the like, and a diol such as ethylene glycol, propylene-1,2-glycol, propylene-1,3-glycol, diethylene glycol, butane-1,4-diol, hexane-1,6-diol, octane-1,8-diol, neopentyl glycol, 2-methyl propane-1,3-diol, or the various isomeric bis-hydroxymethylcyclohexanes; b) a polylactone such as polymers of ε-caprolactone and one of the above mentioned diols; c) a polycarbonate obtained, for example, by reacting one of the above-mentioned diols with diaryl

carbonates or phosgene; or d) a polyether such as a polymer or copolymer of styrene oxide, propylene oxide, tetrahydrofuran, butylene oxide or epichlorohydrin;

$R_3$  is a phosphonate, carboxylate or sulfonate group; and.

$R_2$  is a diamine or diol having a molecular weight less than about 500. Suitable well known diamine chain extenders useful herein include ethylene diamine, diethylene triamine, propylene diamine, butylene diamine, hexamethylene diamine, cyclohexylene diamine, phenylene diamine, tolylene diamine, xylylene diamine, 3,3'-dinitrobenzidine, ethylene methylenebis(2-chloroaniline), 3,3'-dichloro-4,4'-biphenyl diamine, 2,6-diaminopyridine, 4,4'-diamino diphenylmethane, and adducts of diethylene triamine with acrylate or its hydrolyzed products. Also included are materials such as hydrazine, substituted hydrazines such as, for example, dimethyl hydrazine, 1,6-hexamethylene-bis-hydrazine, carbodihydrazide, hydrazides of dicarboxylic acids and sulfonic acids such as adipic acid mono- or dihydrazide, oxalic acid dihydrazide, isophthalic acid dihydrazide, tartaric acid dihydrazide, 1,3-phenylene disulfonic acid dihydrazide, omega-amino-caproic acid dihydrazide, hydrazides made by reacting lactones with hydrazine such as gamma-hydroxybutyric hydrazide, bis-semicarbazide, bis-hydrazide carbonic esters of glycols such as any of the glycols mentioned above. Suitable well known diol chain extenders may be any of the glycols or diols listed above for A.  $R_3$  is a phosphonate, carboxylate or sulfonate group.

The number of repeating units of Structure I can range from 2 to 200, preferably 20 to 100. The amount of the hard-segment (in the right-hand parenthesis) is preferably 40 to 70 percent by weight. The weight ratio of the  $OR_3O$  to the  $OR_2O$  repeating unit preferably varies from 0 to 0.1. The water-dispersible polyurethane employed in the invention may be prepared as described in "Polyurethane Handbook," Hansen Publishers, Munich Vienna, 1985.

The term "polyurethane", as used herein, includes branched and unbranched copolymers, as well as IPN and semi-IPNs comprising at least two polymers, at least one of which is a polyurethane.

An IPN is an intimate combination of two or two or more polymers in a network, involving essentially (that may essentially involve) no covalent bonds or grafts between them. Instead, these intimate mixtures of polymers are held together by permanent entanglements produced when at least one of the polymers is synthesized in the presence of the other. Since there is usually molecular interpenetration of the polymers in IPNs, they tend to phase separate less compared to blends. Such interpenetrating polymer network systems and developments are described by L. H. Sperling in "Interpenetrating Polymer Networks and Related Materials," Plenum Press, New York, 1981, in pages 21-56 of "Multicomponent Polymer Materials" ACS Adv. In Chem. No. 211, edited by D. R. Paul and L. H. Sperling, ACS Books, Washington, D.C., 1986, and in pages 423-436 of "Comprehensive Polymer Science", Volume 6, "Polymer Reactions", edited by G. C. Eastmond, A. Ledwith, S. Russo, and P. Sigwalt, Pergamon Press, Elmsford, N.Y., 1989. While an ideal structure may involve optimal interpenetration, it is recognized that in practice phase separation may limit actual molecular interpenetration. Thus, an IPN may be described as having "interpenetrating phases" and/or "interpenetrating networks." If the synthesis or crosslinking of two or more of the constituent components is concurrent, the system may be designated a simul-

taneous interpenetrating network. If on the other hand, the synthesis and/or crosslinking are carried out separately, the system may be designated a sequential interpenetrating polymer network. A polymer system comprising two or 5 more constituent polymers in intimate contact, wherein at least one is crosslinked and at least one other is linear is designated a semi-interpenetrating polymer network. For example, this type of polymer system has been formed in cured photopolymerizable systems such as disclosed in 10 Chapter 7 of "Imaging Processes and Materials-Nebblette's Eighth Edition," edited by J. M. Sturge, V. Walworth & A. Shepp, Van Nostrand Reinhold, New York, 1989.

In one embodiment of the present invention, the water-dispersible polymer is a polyurethane containing pH responsive groups such as acid functionalities and have an acid number greater than or equal to 5, preferably less than or equal to 40, more preferably less than or equal to 30, most preferably from 10 to 25. The weight ratio of the optional vinyl polymer in the polymer can vary from 0 to 80 percent, 15 including a interpenetrating network of a urethane polymer and a vinyl polymer if the amount of vinyl polymer is substantially greater than zero.

In another embodiment of the present invention, the water-dispersible polymer is a polyurethane-containing 20 component that is an IPN or semi-IPN comprising a polyurethane and a vinyl polymer. By the term "vinyl polymer" is meant an addition polymer that is the reaction product of ethylenically unsaturated monomers. Particularly preferred vinyl polymers are acrylics. Vinyls, especially acrylics, have 25 the added advantage of good adhesion, non-yellowing, are adjustable for high gloss, and have a wide range of glass transition and minimum film forming temperatures. Polymerization of vinyl monomers in the presence of the polyurethane copolymer causes the two polymers to reside in the 30 same latex particle as an interpenetrating or semi-interpenetrating network particle resulting in improved resistance to water, organic solvents and environmental conditions, improved tensile strength, and modulus of elasticity. The presence of groups such as carboxylic acid groups 35 provide a conduit for processing solutions to permeate the coating at pH greater than 7. Preferably, the acid number is maintained at less than or equal to 40 to ensure that overcoat has good adhesion to the substrate below, even at high pH, and makes the overcoat more water-resistant.

A preferred IPN comprises an interpenetrating polyurethane and vinyl polymer. Such an IPN is also sometimes referred to in the trade as a urethane-vinyl copolymer or hybrid copolymer, even though involving essentially no chemical bonds between the two polymer chains. Such an 40 IPN may be conventionally produced by polymerizing one or more vinyl monomers in the presence of the polyurethane prepolymer or a chain extended polyurethane. It is possible to have more than two polymers or for each of the polymer chains to be branched or linear. Suitably, in such an IPN, the 45 weight ratio of polyurethane component to vinyl component is 1:20 to 20:1. The preferred weight ratio of the polyurethane to the vinyl component is about 4:1 to about 1:4, more preferably about 1:1 to 1:4.

Preferably, the polyurethane has an acid number of greater 50 than or equal to 5, preferably less than or equal to 40, more preferably less than or equal to 30. Acid number is in general determined by titration and is defined as the number of milligrams of potassium hydroxide (KOH) required to neutralize 1 gram of the polymer.

Preparation of an aqueous dispersion of a polyurethane-containing component, when a single copolymer, is well known in the art. In a preferred method of preparation, the

first step is the formation of a medium molecular weight isocyanate terminated prepolymer by the reaction of suitable di or polyol with a stoichiometric excess of di or polyisocyanates. The prepolymer is then generally dispersed in water via water-solubilizing/dispersing groups that are introduced either into the prepolymer prior to chain extension, or are introduced as part of the chain extension agent. Therefore, small particle size stable dispersions can frequently be produced without the use of an externally added surfactant. The prepolymer in the aqueous solution is then subjected to chain extension using diamines or diols to form the "fully reacted" polyurethane.

When a vinyl polymer is present in the polyurethane-containing component, such urethane-vinyl IPN copolymers may be produced, for example, by polymerizing one or more vinyl monomers in the presence of the polyurethane prepolymer or the chain extended polyurethane. The preferred weight ratio of the chain extended polyurethane to the vinyl monomer being about 4:1 to about 1:4, most preferably about 1:1 to 1:4, as mentioned above.

Polyols useful for the preparation of polyurethane dispersions of the present invention include polyester polyols prepared from one or more diols (e.g. ethylene glycol, butylene glycol, neopentyl glycol, hexane diol or mixtures of any of the above) and one or more dicarboxylic acids or anhydrides (succinic acid, adipic acid, suberic acid, azelaic acid, sebatic acid, phthalic acid, isophthalic acid, maleic acid and anhydrides of these acids), polylactone diols prepared from lactones such as caprolactone reacted with a diol, polyesteramides containing polyols prepared by inclusion of amino-alcohols such as ethanol amine during the polyesterification process, polyether polyols prepared from for example, ethylene oxide, propylene oxide or tetrahydrofuran, polycarbonate polyols prepared from reacting diols with diaryl carbonates, and hydroxyl terminated polyolefins prepared from ethylenically unsaturated monomers. Combinations of such polyols are also useful. As mentioned below, polysiloxane polyols are also useful in forming a polyurethane. See, for example, U.S. Pat. No. 5,876,981 to Anderson, hereby incorporated by reference, for such monomers. A polyester polyol is preferred for the present invention.

Polyisocyanates useful for making the prepolymer may be aliphatic, aromatic or araliphatic. Examples of suitable polyisocyanates include one or more of the following: toluene diisocyanate, tetramethylene diisocyanate, hexamethylene diisocyanate, isophorone diisocyanate, ethylethylene diisocyanate, 2,3-dimethylethylene diisocyanate, 1-methyltrimethylene diisocyanate, 1,3-cyclopentylene diisocyanate, 1,4-cyclohexylene diisocyanate, 1,3-phenylene diisocyanate, 4,4'-biphenylene diisocyanate, 1,5-naphthalene diisocyanate, bis-(4-isocyanato cyclohexyl)-methane, 4,4'-diisocyanato diphenyl ether, tetramethyl xylene diisocyanate, polymethylene polyphenyl polyisocyanates and the like. Methylene bis(isocyanato cyclohexane) is preferred.

Preferably, a suitable portion of the prepolymer also contains at least one comparatively unreactive pendant carboxylic group, in salt form or preferably neutralized with a suitable basic material to form a salt during or after prepolymer formation or during formation of the dispersion. This helps provide permeability of processing solutions through the overcoat at pHs greater than 7 and dispersibility in water. Suitable compounds that are reactive with the isocyanate groups and have a group capable of forming an anion include, but are not limited to the following: dihydroxypropionic acid, dimethylolpropionic acid, dihydrox-

ysuccinic acid and dihydroxybenzoic acid. Other suitable compounds are the polyhydroxy acids which can be prepared by oxidizing monosaccharides, for example gluconic acid, saccharic acid, mucic acid, glucuronic acid and the like. Such a carboxylic-containing reactant is preferably an  $\alpha,\alpha$ -dimethylolalkanoic acid, especially 2,2-dimethylol propionic acid.

Suitable tertiary amines which may be used to neutralize the acid and form anionic groups for water dispersability are trimethylamine, triethylamine, dimethylaniline, diethylaniline, triphenylamine and the like.

Chain extenders suitable for optionally chain extending the prepolymer are, for example, active-hydrogen containing molecules such as polyols, amino alcohols, ammonia, primary or secondary aliphatic, aromatic, alicyclic araliphatic or heterocyclic amines especially diamines. Diamines suitable for chain extension of the pre-polyurethane include ethylenediamine, diaminopropane, hexamethylene diamine, hydrazine, aminoethyl ethanolamine and the like.

In accordance with one embodiment of this invention, a urethane-vinyl IPN may be prepared by polymerizing vinyl addition monomers in the presence of the polyurethane prepolymer or the chain extended polyurethane. The solution of the water-dispersible polyurethane prepolymer in vinyl monomer may be produced by dissolving the prepolymer in one or more vinyl monomers before dispersing the prepolymer in water.

Suitable vinyl monomers in which the prepolymer may be dissolved contain one or more polymerizable ethylenically unsaturated groups. Preferred monomers are liquid under the temperature conditions of prepolymer formation, although the possibility of using solid monomers in conjunction with organic solvents is not excluded.

The vinyl polymers useful for the present invention include those obtained by copolymerizing one or more ethylenically unsaturated monomers including, for example, alkyl esters of acrylic or methacrylic acid such as methyl methacrylate, ethyl methacrylate, butyl methacrylate, ethyl acrylate, butyl acrylate, hexyl acrylate, n-octyl acrylate, lauryl methacrylate, 2-ethylhexyl methacrylate, nonyl acrylate, benzyl methacrylate, the hydroxyalkyl esters of the same acids such as 2-hydroxyethyl acrylate, 2-hydroxyethyl methacrylate, and 2-hydroxypropyl methacrylate, the nitrile and amides of the same acids such as acrylonitrile, methacrylonitrile, and methacrylamide, vinyl acetate, vinyl propionate, vinylidene chloride, vinyl chloride, and vinyl aromatic compounds such as styrene, t-butyl styrene and vinyl toluene, dialkyl maleates, dialkyl itaconates, dialkyl methylene-malonates, isoprene, and butadiene. Suitable ethylenically unsaturated monomers containing carboxylic acid groups include acrylic monomers such as acrylic acid, methacrylic acid, ethacrylic acid, itaconic acid, maleic acid, fumaric acid, monoalkyl itaconate including monomethyl itaconate, monoethyl itaconate, and monobutyl itaconate, monoalkyl maleate including monomethyl maleate, monoethyl maleate, and monobutyl maleate, citraconic acid, and styrene carboxylic acid. Suitable polyethylenically unsaturated monomers include butadiene, isoprene, allylmethacrylate, diacrylates of alkyl diols such as butane-1,3-diol diacrylate and hexanediol diacrylate, divinyl benzene and the like.

The prepolymer/vinyl monomer solution may be dispersed in water using techniques well known in the art. Preferably, the solution is added to water with agitation or, alternatively, water may be stirred into the solution. Polymerization of the vinyl monomer or monomers is brought about by free radical initiators at elevated temperatures.

Free radicals of any sort may be used including persulfates (such as ammonium persulfate, potassium persulfate, etc., peroxides (such as hydrogen peroxide, benzoyl peroxide, cumene hydroperoxide, tertiary butyl peroxide, etc.), azo compounds (such as azobiscyanovaleric acid, azoisobutyronitrile, etc.), and redox initiators (such as hydrogen peroxide-iron(II) salt, potassium persulfate-sodium hydrogen sulfate, etc.). Preferable free radical initiators are the ones that partition preferably into the oil phase such as the azo-type initiators. Common chain transfer agents or mixtures thereof known in the art, such as alkyl-mercaptans, can be used to control the polymer molecular weight.

Polymerization may be carried out by various methods. In one method, all of the vinyl monomer (the same or different vinyl monomers or monomer mixtures) is added in order to swell the polyurethane prepolymer. The monomers are then polymerized using an oil soluble free radical initiator after dispersing the mixture in water.

In a second alternative method, some of vinyl monomer may be added to swell the pre-polymer prior to dispersing in water. The rest of the monomer is fed into the system during the polymerization process. Other methods include feeding in all the vinyl monomer during the copolymerization process.

Some examples of polyurethane-containing components used in the practice of this invention that are commercially available include NeoPac® R-9000, R-9699 and R-9030 from NeoResins (Wilmington, Del.), Sancure® AU4010 from BF Goodrich (Akron, Ohio), and Flexthane® 620, 630, 790 and 791 from Air Products. An example of the polyurethane-containing copolymer useful in the practice that is commercially available is the NeoRez® R9679.

In another embodiment of the invention, the water-dispersible polymer is an essentially hydrophobic, substantially amorphous, thermoplastic polyester polymer in which 30 ionic groups or moieties are present in sufficient number to provide water dispersibility prior to coating. The polyester dispersions provide advantageous properties such as good film-formation, good chemical-resistance, wet-abrasion resistance, excellent fingerprint resistance, toughness, elasticity and durability. Furthermore, the polyesters exhibit tensile and flexural strength and resistance to various oils.

Procedures for the preparation of polyester ionomers are described in U.S. Pat. Nos. 3,018,272; 3,563,942; 3,734, 45 874; 3,779,993; 3,929,489; 4,307,174, 4,395,475, 5,939,355 and 3,929,489, the disclosures of which are incorporated herein by reference. The substantially amorphous polyesters useful in this invention comprise dicarboxylic acid recurring units typically derived from dicarboxylic acids or their 50 functional equivalents and diol recurring units typically derived from diols. Generally, such polyesters are prepared by reacting one or more diols with one or more dicarboxylic acids or their functional equivalents (e.g. anhydrides, diesters or diacid halides), as described in detail in the cited patents. Such diols, dicarboxylic acids and their functional equivalents are sometimes referred to in the art as polymer precursors. It should be noted that, as known in the art, carbonylimino groups can be used as linking groups rather than carboxyloxy groups. This modification is readily achieved by reacting one or more diamines or amino alcohols with one or more dicarboxylic acids or their functional equivalents. Mixtures of diols and diamines can be used if desired.

Conditions for preparing the polyesters useful in this 65 invention are known in the art as described above. The polymer precursors are typically, condensed in a ratio of at

least 1 mole of diol for each mole of dicarboxylic acid in the presence of a suitable catalyst at a temperature of from about 125° to about 300° C. Condensation pressure is typically from about 0.1 mm Hg to about one or more atmospheres. 5 Low-molecular weight by-products can be removed during condensation, e.g. by distillation or another suitable technique. The resulting condensation polymer is polycondensed under appropriate conditions to form a polyester. Polycondensation is usually carried out at a temperature of from about 150° to about 300° C. and a pressure very near vacuum, although higher pressures can be used.

Polyester ionomers, useful in the present composition, contain at least one ionic moiety, which can also be referred to as an ionic group, functionality, or radical. In a preferred embodiment of the invention, the recurring units containing 15 ionic groups are present in the polyester ionomer in an amount of from about 1 to about 12 mole percent, based on the total moles of recurring units. Such ionic moieties can be provided by either ionic diol recurring units and/or ionic dicarboxylic acid recurring units, but preferably by the latter. Such ionic moieties can be anionic or cationic in nature, but preferably, they are anionic. Exemplary anionic ionic groups include carboxylic acid, sulfonic acid, and disulfonylimino 20 and their salts and others known to a worker of ordinary skill in the art. Sulfonic acid ionic groups, or salts thereof, are preferred.

One type of ionic acid component has the structure



where M=H, Na, K or NH<sub>4</sub>.

Ionic dicarboxylic acid recurring units can be derived 30 from 5-sodiosulfobenzene-1,3-dicarboxylic acid, 5-sodiosulfocyclohexane-1,3-dicarboxylic acid, 5-(4-sodiosulfophenoxy)benzene-1,3-dicarboxylic acid, 5-(4-sodiosulfophenoxy)cyclohexane-1,3-dicarboxylic acid, similar compounds and functional equivalents thereof and others described in U.K. Patent Specification No. 1,470,059 (published Apr. 14, 1977). Other suitable polyester ionomers for protective overcoats in the imaged elements of the present invention are disclosed in U.S. Pat. Nos. 4,903,039 and 4,903,040, which are incorporated herein by reference.

Another type of ionic dicarboxylic acid found useful in the practice of this invention are those having units represented by the formula:



wherein each of m and n is 0 or 1 and the sum of m and n 60 is 1; each X is carbonyl; Q has the formula:



Q' has the formula:



Y is a divalent aromatic radical, such as arylene (e.g. phenylene, naphthalene, xylylene, etc.) or arylidyne (e.g. phenenyl, naphthylidyne, etc.); Z is a monovalent aromatic radical, such as aryl, aralkyl or alkaryl (e.g. phenyl, p-methylphenyl, naphthyl, etc.), or alkyl having from 1 to 12 carbon atoms, such as methyl, ethyl, isopropyl, n-pentyl, neopentyl, 2-chlorohexyl, etc., and preferably from 1 to 6 carbon atoms; and M is a solubilizing cation and preferably a monovalent cation such as an alkali metal or ammonium cation.

The hydrophilic polymer according to the present invention can include gelatin if substantially non-crosslinked. For example, in one embodiment of the invention, the overcoat is applied to the imaging element as a composition comprising 10 to 50% by weight gelatin and 50 to 90% by weight of water-dispersible particles (by weight of dry laydown of the entire overcoat) having an average diameter of 10 to 500 nm. Since gelatin comprises a substantial portion of the overcoat layer, photographic elements containing this overcoat are readily manufactured using conventional photographic coating equipment. A proteolytic enzyme can be applied to the element in reactive association with the overcoat layer. The layer containing the overcoat polymer and the enzyme can be applied either in the same coating operation (using a slide hopper or other means of applying multiple layers) at the same time with the imaging layer, in a sequential coating operation (using a separate coating station) with the imaging layer, or in a separate coating operation (at a later time to an element having at least one previously applied, dried, and hardened imaging layer), to produce a photographic element comprising a gelatin-containing overcoat. Typically, the gelatin in the overcoat layer is substantially hydrolyzed or degraded (digested) by the enzyme before the photochemical processing of the imaged element. Advantageously, a photographic element according to one embodiment of the invention can be exposed and processed using normal photofinishing equipment, with no modifications, to provide an imaged element that possesses a protective, water-resistant layer. Further details of such an enzyme containing imaging element is described in commonly assigned U.S. Ser. No. 09/564,598, herein incorporated by reference in its entirety.

The protective overcoat should be clear, i.e., transparent, and is preferably colorless. But it is specifically contemplated that the polymer overcoat can have some color for the purposes of color correction, or for special effects, so long as it does not detrimentally affect the formation or viewing of the image through the overcoat. Thus, there can be incorporated into the polymer a dye that will impart color or tint. In addition, additives can be incorporated into the polymer that will give the overcoat various desired properties. For example, a UV absorber may be incorporated into the polymer to make the overcoat UV absorptive, thus protecting the image from UV induced fading. Other compounds may be added to the coating composition, depending on the functions of the particular layer, including surfactants, emulsifiers, coating aids, lubricants, matte particles, rheology modifiers, crosslinking agents, antifoggants, inorganic fillers such as conductive and nonconductive metal oxide particles, pigments, magnetic particles, biocide, and the like.

The coating composition may also include a small amount of organic solvent, preferably the concentration of organic solvent is less than 1 percent by weight of the total coating composition. The invention does not preclude coating the desired polymeric material from a volatile organic solution or from a melt of the polymer.

Examples of coating aids include surfactants, viscosity modifiers and the like. Surfactants include any surface-active material that will lower the surface tension of the 10 coating preparation sufficiently to prevent edge-withdrawal, repellencies, and other coating defects. These include alkyloxy- or alkylphenoxy polyether or polyglycidol derivatives and their sulfates, such as nonylphenoxy poly(glycidol) available from Olin Matheson Corporation or sodium 15 octylphenoxy poly(ethyleneoxide) sulfate, organic sulfates or sulfonates, such as sodium dodecyl sulfate, sodium dodecyl sulfonate, sodium bis(2-ethylhexyl)sulfosuccinate (Aerosol OT), and alkylcarboxylate salts such as sodium decanoate.

The surface characteristics of the overcoat are in large part 20 dependent upon the physical characteristics of the polymers which form the continuous phase and the presence or absence of solid, non fusible particles. However, the surface characteristics of the overcoat also can be modified by the 25 conditions under which the surface is optionally fused. For example, in contact fusing, the surface characteristics of the fusing element that is used to fuse the polymers to form the continuous overcoat layer can be selected to impart a desired degree of smoothness, texture or pattern to the surface of the 30 element. Thus, a highly smooth fusing element will give a glossy surface to the imaged element, a textured fusing element will give a matte or otherwise textured surface to the element, a patterned fusing element will apply a pattern to the surface of the element, etc.

35 Matte particles well known in the art may also be used in the coating composition of the invention, such matting agents have been described in *Research Disclosure* No. 308119, published December 1989, pages 1008 to 1009. When polymer matte particles are employed, the polymer 40 may contain reactive functional groups capable of forming covalent bonds with the binder polymer by intermolecular crosslinking or by reaction with a crosslinking agent in order to promote improved adhesion of the matte particles to the 45 coated layers. Suitable reactive functional groups include hydroxyl, carboxyl, carbodiimide, epoxide, aziridine, vinyl sulfone, sulfonic acid, active methylene, amino, amide, allyl, and the like.

In order to reduce the sliding friction of the photographic 50 elements in accordance with this invention, the water-dispersible polymers may contain fluorinated or siloxane-based components and/or the coating composition may also include lubricants or combinations of lubricants. Typical lubricants include (1) silicone based materials disclosed, for example, in U.S. Pat. Nos. 3,489,567, 3,080,317, 3,042,522, 4,004,927, and 4,047,958, and in British Patent Nos. 955, 061 and 1,143,118; (2) higher fatty acids and derivatives, higher alcohols and derivatives, metal salts of higher fatty acids, higher fatty acid esters, higher fatty acid amides, polyhydric alcohol esters of higher fatty acids, etc., disclosed in U.S. Pat. Nos. 2,454,043; 2,732,305; 2,976,148; 3,206,311; 3,933,516; 2,588,765; 3,121,060; 3,502,473; 3,042,222; and 4,427,964, in British Patent Nos. 1,263,722; 1,198,387; 1,430,997; 1,466,304; 1,320,757; 1,320,565; and 1,320,756; and in German Patent Nos. 1,284,295 and 1,284, 294; (3) liquid paraffin and paraffin or wax like materials such as carnauba wax, natural and synthetic waxes, petroleum waxes, mineral waxes, silicone-wax copolymers and

the like; (4) perfluoro- or fluoro- or fluorochloro-containing materials, which include poly(tetrafluoroethylene), poly(trifluorochloroethylene), poly(vinylidene fluoride, poly(trifluorochloroethylene-co-vinyl chloride), poly(meth)acrylates or poly(meth)acrylamides containing perfluoroalkyl side groups, and the like. Lubricants useful in the present invention are described in further detail in *Research Disclosure* No.308119, published December 1989, page 1006.

The support material used with this invention can comprise various polymeric films, papers, glass, and the like. The thickness of the support is not critical. Support thicknesses of 2 to 15 mils (0.002 to 0.015 inches) can be used. Biaxially oriented support laminates can be used with the present invention. These supports are disclosed in commonly owned U.S. Pat. Nos. 5,853,965, 5,866,282, 5,874, 205, 5,888,643, 5,888,681, 5,888,683, and 5,888,714, incorporated in their entirety by reference herein. These supports include a paper base and a biaxially oriented polyolefin sheet, typically polypropylene, laminated to one or both sides of the paper base. At least one photosensitive silver halide layer is applied to the biaxially oriented polyolefin sheet.

The coating composition of the invention can be applied by any of a number of well known techniques, such as dip coating, rod coating, blade coating, air knife coating, gravure coating and reverse roll coating, extrusion coating, slide coating, curtain coating, and the like. After coating, the layer is generally dried by simple evaporation, which may be accelerated by known techniques such as convection heating. Known coating and drying methods are described in further detail in *Research Disclosure* No. 308119, Published December 1989, pages 1007 to 1008. Preferably, a commercial embodiment involve simultaneous co-extrusion.

The laydown of the overcoat will depend on its field of application. For a photographic element, the laydown of the polyurethane-containing copolymer is suitably at least 0.54 g/m<sup>2</sup> (50 mg/ft<sup>2</sup>), preferably 1.08 to 5.38 g/m<sup>2</sup> (100 to 500 mg/ft<sup>2</sup>), most preferably 1.61 to 3.23 g/m<sup>2</sup>(150 to 300 mg/ft<sup>2</sup>). It may be advantageous to increase the amount of polyvinyl alcohol in the overcoat as the laydown increases in order to improve the developability.

After applying the coating composition to the support, it may be dried over a suitable period of time, for example 2 to 4 minutes. In the event of cracking, especially at lower levels of polyvinyl alcohol or when using an alternative film-forming polymer, it may be advantageous to adjust the temperature and/or humidity of the drying step to eliminate or reduce this cracking problem. Without wishing to be bound by theory, it is believed that higher levels of polyvinyl alcohol with limited degree of hydrolysis reduces the tendency of the polyvinyl alcohol to block the release of water during drying, which might otherwise occur with overly fast film formation and drying. Thus, polyvinyl alcohol according to one embodiment of the invention, by delaying film formation allows the release of water during drying which if blocked might otherwise adversely affect the uniformity of the overcoat.

Photographic elements can contain conductive layers incorporated into multilayer photographic elements in any of various configurations depending upon the requirements of the specific photographic element. Preferably, the conductive layer is present as a subbing or tie layer underlying a magnetic recording layer on the side of the support opposite the photographic layer(s). However, conductive layers can be overcoated with layers other than a transparent magnetic recording layer (e.g., abrasion-resistant backing layer, curl

control layer, pelloid, etc.) in order to minimize the increase in the resistivity of the conductive layer after overcoating. Further, additional conductive layers also can be provided on the same side of the support as the photographic layer(s) or on both sides of the support. An optional conductive subbing layer can be applied either underlying or overlying a gelatin subbing layer containing an antihalation dye or pigment. Alternatively, both antihalation and antistatic functions can be combined in a single layer containing conductive particles, antihalation dye, and a binder. Such a hybrid layer is typically coated on the same side of the support as the sensitized emulsion layer. Additional optional layers can be present as well. An additional conductive layer can be used as an outermost layer of an photographic element, for example, as a protective layer overlying an image-forming layer. When a conductive layer is applied over a sensitized emulsion layer, it is not necessary to apply any intermediate layers such as barrier or adhesion-promoting layers between the conductive overcoat layer and the photographic layer(s), although they can optionally be present. Other addenda, such as polymer lattices to improve dimensional stability, hardeners or cross-linking agents, surfactants, matting agents, lubricants, and various other well-known additives can be present in any or all of the above mentioned layers.

Conductive layers underlying a transparent magnetic recording layer typically exhibit an internal resistivity of less than  $1 \times 10^{10}$  ohms/square, preferably less than  $1 \times 10^9$  ohms/square, and more preferably, less than  $1 \times 10^8$  ohms/square.

Photographic elements of this invention can differ widely in structure and composition. For example, the photographic elements can vary greatly with regard to the type of support, the number and composition of the image-forming layers, and the number and types of auxiliary layers that are included in the elements. In particular, photographic elements can be still films, motion picture films, x-ray films, graphic arts films, paper prints or microfiche. It is also specifically contemplated to use the conductive layer of the present invention in small format films as described in *Research Disclosure*, Item 36230 (June 1994). Photographic elements can be either simple black-and-white or monochrome elements or multilayer and/or multicolor elements adapted for use in a negative-positive process or a reversal process. Generally, the photographic element is prepared by coating one side of the film support with one or more layers comprising a dispersion of silver halide crystals in an aqueous solution of gelatin and optionally one or more subbing layers. The coating process can be carried out on a continuously operating coating machine wherein a single layer or a plurality of layers are applied to the support. For multicolor elements, layers can be coated simultaneously on the composite film support as described in U.S. Pat. Nos. 2,761,791 and 3,508,947. Additional useful coating and drying procedures are described in *Research Disclosure*, Vol. 176, Item 17643 (December, 1978).

Photographic elements protected in accordance with this invention may be derived from silver-halide photographic elements that can be black and white elements (for example, those which yield a silver image or those which yield a neutral tone image from a mixture of dye forming couplers), single color elements or multicolor elements. Multicolor elements typically contain dye image-forming units sensitive to each of the three primary regions of the spectrum. The imaged elements can be imaged elements which are viewed by transmission, such a negative film images, reversal film images and motion-picture prints or they can be imaged elements that are viewed by reflection, such a paper prints. Because of the amount of handling that can occur with paper

prints and motion picture prints, they are the preferred imaged photographic elements for use in this invention.

While a primary purpose of applying an overcoat to imaged elements in accordance with this invention is to protect the element from physical damage, application of the overcoat may also protect the image from fading or yellowing. This is particularly true with elements that contain images that are susceptible to fading or yellowing due to the action of oxygen. For example, the fading of dyes derived from pyrazolone and pyrazoloazole couplers is believed to be caused, at least in part, by the presence of oxygen, so that the application of an overcoat which acts as a barrier to the passage of oxygen into the element will reduce such fading.

Photographic elements in which the images to be protected are formed can have the structures and components shown in Research Disclosures 37038 and 38957. Other structures which are useful in this invention are disclosed in commonly owned U.S. Ser. No. 09/299,395, filed Apr. 26, 1999 and U.S. Ser. No. 09/299,548, filed Apr. 26, 1999, incorporated in their entirety by reference. Specific photographic elements can be those shown on pages 96-98 of Research Disclosure 37038 as Color Paper Elements 1 and 2. A typical multicolor photographic element comprises a support bearing a cyan dye image-forming unit comprised of at least one red-sensitive silver halide emulsion layer having associated therewith at least one cyan dye-forming coupler, a magenta dye image-forming unit comprising at least one green-sensitive silver halide emulsion layer having associated therewith at least one magenta dye-forming coupler, and a yellow dye image-forming unit comprising at least one blue-sensitive silver halide emulsion layer having associated therewith at least one yellow dye-forming coupler.

The photographic element can contain additional layers, such as filter layers, interlayers, overcoat layers, subbing layers, and the like. All of these can be coated on a support that can be transparent (for example, a film support) or reflective (for example, a paper support). Photographic elements protected in accordance with the present invention may also include a magnetic recording material as described in *Research Disclosure*, Item 34390, November 1992, or a transparent magnetic recording layer such as a layer containing magnetic particles on the underside of a transparent support as described in U.S. Pat. Nos. 4,279,945 and 4,302,523.

Suitable silver-halide emulsions and their preparation, as well as methods of chemical and spectral sensitization, are described in Sections I through V of Research Disclosures 37038 and 38957. Others are described in U.S. Ser. No. 09/299,395, filed April 26, 1999 and U.S. Ser. No. 09/299,548, filed Apr. 26, 1999, which are incorporated in their entirety by reference herein. Color materials and development modifiers are described in Sections V through XX of Research Disclosures 37038 and 38957. Vehicles are described in Section II of Research Disclosures 37038 and 38957, and various additives such as brighteners, antifoggants, stabilizers, light absorbing and scattering materials, hardeners, coating aids, plasticizers, lubricants and matting agents are described in Sections VI through X and XI through XIV of Research Disclosures 37038 and 38957. Processing methods and agents are described in Sections XIX and XX of Research Disclosures 37038 and 38957, and methods of exposure are described in Section XVI of Research Disclosures 37038 and 38957.

Photographic elements typically provide the silver halide in the form of an emulsion. Photographic emulsions generally include a vehicle for coating the emulsion as a layer of a photographic element. Useful vehicles include both natu-

rally occurring substances such as proteins, protein derivatives, cellulose derivatives (e.g., cellulose esters), gelatin (e.g., alkali-treated gelatin such as cattle bone or hide gelatin, or acid treated gelatin such as pigskin gelatin), gelatin derivatives (e.g., acetylated gelatin, phthalated gelatin, and the like). Also useful as vehicles or vehicle extenders are hydrophilic water-permeable colloids. These include synthetic polymeric peptizers, carriers, and/or binders such as poly(vinyl alcohol), poly(vinyl lactams), acrylamide polymers, polyvinyl acetals, polymers of alkyl and sulfoalkyl acrylates and methacrylates, hydrolyzed polyvinyl acetates, polyamides, polyvinyl pyridine, methacrylamide copolymers, and the like.

Photographic elements can be imagewise exposed using a variety of techniques. Typically exposure is to light in the visible region of the spectrum, and typically is of a live image through a lens. Exposure can also be to a stored image (such as a computer stored image) by means of light emitting devices (such as LEDs, CRTs, etc.).

Images can be developed in photographic elements in any of a number of well known photographic processes utilizing any of a number of well known processing compositions, described, for example, in T. H. James, editor, *The Theory of the Photographic Process*, 4th Edition, Macmillan, New York, 1977. In the case of processing a color negative element, the element is treated with a color developer (that is one which will form the colored image dyes with the color couplers), and then with an oxidizer and a solvent to remove silver and silver halide. In the case of processing a color reversal element, the element is first treated with a black and white developer (that is, a developer which does not form colored dyes with the coupler compounds) followed by a treatment to render developable unexposed silver halide (usually chemical or light fogging), followed by treatment with a color developer. Development is followed by bleaching, fixing, to remove silver or silver halide, washing and drying.

In one embodiment of a method of using a composition according to the present invention, a photographic element may be provided with a processing-solution-permeable overcoat having the above described composition overlying the silver halide emulsion layer superposed on a support. The photographic element is developed in an alkaline developer solution having a pH greater than 7, preferably greater than 8, more preferably greater than 9. This allows the developer to penetrate the protective coating. After the pH is reduced, for example in a bleach fix solution, the protective overcoat becomes relatively water resistant. The addition of polyvinyl alcohol, according to one embodiment of the present invention, facilitates this method. It has been found the polyvinyl alcohol can provide improved wettability of the surface during processing and, at the same time, allows more of the polyvinyl alcohol to be washed out during the processing, so that the final product is more water resistant. Suitably at least 30%, preferably greater than 50%, more preferably greater than 75% of the original amount of PVA in the overcoat is washed out during processing of the exposed photographic element, such that the final product is depleted in hydrophilic polymer and hence relatively more water resistant. Although the processing-solution-permeable overcoat does not require fusing, optional fusing may improve the water resistance further.

The overcoat layer in accordance with this invention is particularly advantageous for use with photographic prints due to superior physical properties including excellent resistance to water-based spills, fingerprinting, fading and yellowing, while providing exceptional transparency and toughness necessary for providing resistance to scratches, abrasion, blocking, and ferrotyping.

The present invention is illustrated by the following examples. Unless otherwise indicated, the molecular weights herein are weight average molecular weights, as determined by size exclusion chromatography described below.

### EXAMPLES

#### Characterization of Polymeric Materials

##### Glass Transition Temperature and Melting Temperature

Both glass transition temperature ( $T_g$ ) and melting temperature ( $T_m$ ) of the dry polymer material were determined by differential scanning calorimetry (DSC), using a ramping rate of 20° C./minute.  $T_g$  is defined herein as the inflection point of the glass transition and  $T_m$  is defined herein as the peak of the melting transition.

##### Particle Size Measurement

All particles were characterized by Photon Correlation Spectroscopy using a Zetasizer Model DTS5100 manufactured by Malvern Instruments.

##### Average Molecular Weight

Polymer samples were analyzed by size-exclusion chromatography in tetrahydrofuran using three Polymer Laboratories Plgel™ mixed-C columns. The column set was calibrated with narrow-molecular-weight distribution polystyrene standards between 595 ( $\log M=2.76$ ) and 2170000 ( $\log M=6.34$ ) daltons. The number average ( $M_n$ ) and weight average ( $M_w$ ) were reported. The poly(vinyl alcohol) samples were analyzed by size-exclusion chromatography (SEC) in dimethyl sulfoxide (DMSO) containing 0.01 M lithium nitrate using one Jordi Gel GBR mixed-bed column. The column set was calibrated with narrow-molecular-weight distribution pullulan standards between MW 5,900 ( $\log M=3.77$ ) and MW 788,000 ( $\log M=5.90$ ). Results were plotted as pullulan equivalent molecular weights and the number average ( $M_n$ ) and weight average ( $M_w$ ) were reported.

##### Polymer Preparation

###### P1 Butyl Methacrylate Latex

To a 1 L three-necked reaction flask fitted with a stirrer and condenser was added 300 ml of degassed distilled water, 2 ml of 45% Dowfax® 2A1, 1.00 grams of potassium persulfate, and 0.33 grams of sodium metabisulfite. The flask was placed in a 60° C. bath and the contents of an addition flask containing 100 ml of distilled water, 2 ml of 45% Dowfax® 2A1, 95 grams of n-butyl methacrylate and 5 grams of 2-sulfo-1,1diethylethyl acrylamide (sodium salt) was added to the reaction flask over a period of 40 minutes. The reaction flask was stirred at 80° C. for 1 hour and 0.25 g of potassium persulfate was added and the contents stirred at 80° C. for additional 90 minutes. The flask was cooled and the pH of the latex was adjusted to 5.5 using 10% sodium hydroxide to give a latex containing 20% solids. The  $T_g$  of the polymer was 35C.

###### P2 Ethyl Acrylate/Vinylidene Chloride/Hydroxyethyl Acrylate Latex (10/88/2)

To a 20-ounce polyethylene bottle was added 341 grams of demineralized water. The water was purged for 15–20 minutes with nitrogen. The following were added to the reactor in order: 5.10 grams of 30% Triton® 770, 3.06 grams of hydroxyethyl acrylate, 15.29 grams of ethyl acrylate, 134.59 grams of vinylidene chloride, 0.7586 grams of potassium metabisulfite, and 0.3794 grams of potassium persulfate. The bottle was capped and placed in a tumbler bath at 40° C., and held there for 16–20 hours. The product was then removed from the bath, and cooled to 20° C. The product was filtered through cheesecloth. Glass transition temperature was 9° C. as measured by DSC, average particle size obtained from PCS was 75 nm.

##### P3 (Polyurethane Dispersion)

In a 1 liter resin flask equipped with thermometer, stirrer, water condenser and a vacuum outlet, melted 75.68 grams (0.088 mole) polycarbonate polyol KM101733 (Mw=860) and dewatered under vacuum at 100° C. Released vacuum and at 40° C. added 10.25 grams (0.076 mole) of dimethylol propionic acid, 30.28 grams (0.336 mole) of 1,4-butanediol, 75 grams of tetrahydrofuran and 15 drops of dibutyltin dilaurate (catalyst) while stirring. Adjusted temperature to 75° C. when a homogeneous solution was obtained, slowly added 111.28 grams (0.50 mole) of isophorone diisocyanate followed by 25 grams of tetrahydrofuran. For this polymer, the monomer feed ratio on a weight basis was 33.3% polycarbonate polyol, 4.5% dimethylol propionic acid, 13.3% butanediol and 48.9% isophorone diisocyanate. After maintaining for about 4 hours to complete the reaction, NCO was substantially nil. Stirred in a stoichiometric amount of potassium hydroxide based on dimethylol propionic acid, and maintained for 5 min. Mixed with 1300 grams of water under high shear to form a stable aqueous dispersion. Tetrahydrofuran was removed by heating under vacuum to give an aqueous dispersion at 19.1% solids. Glass transition temperature was 53° C. as measured by DSC, weight average molecular weight was 11,000 and particle size was 30nm.

##### P4 (Polyurethane Dispersion)

The same preparation scheme was used as for P3 except diethylene glycol was substituted for a portion of the 1,4-butanediol as chain extender, such that the monomer feed ratio on a weight basis was 33.0% polycarbonate polyol, 4.4% dimethylol propionic acid, 9.5% butanediol, 4.3% diethylene glycol and 48.9% isophorone diisocyanate. Tetrahydrofuran was removed by heating under vacuum to give an aqueous dispersion at 19.5% solids. Glass transition temperature was 55° C. as measured by DSC, and weight average molecular weight was 19,100.

##### P5 (Polyurethane Dispersion)

The same preparation scheme was used as for P3 except diethylene glycol was substituted for a portion of the 1,4-butanediol and the relative amounts of other components were adjusted such that the monomer feed ratio on a weight basis was 44.3% polycarbonate polyol, 4.6% dimethylol propionic acid, 6.5% butanediol, 3.6% diethylene glycol and 43.0% isophorone diisocyanate. Tetrahydrofuran was removed by heating under vacuum to give an aqueous dispersion at 25.3% solids. Glass transition temperature was 33° C. as measured by DSC, and weight average molecular weight was 12,600.

##### P6 (Polyurethane-Acrylic Copolymer Dispersion)

Into a dry reactor was charged 96 grams of a diol (Millester® 9-55, MW2000 from Polyurethane Corporation of America), 87 grams of the methylene bis(4-cyclohexyl) isocyanate (Desmodur®W) and 0.02 grams of dibutyltin dilaurate (Aldrich). The mixture was held with stirring for 90 minutes at 94° C. under a blanket of argon after which 14 grams of dimethylol propionic acid was added to the reactor and the mixture stirred for 1.5 hours at 94° C. At this point 24 grams of methyl methacrylate were added and stirred for 1 hour at the same temperature. The resultant prepolymer was cooled to below 40° C., dissolved in a vinyl monomer mixture consisting of 113 grams of n-butyl acrylate, 183 grams of methyl methacrylate, and 5 grams of acetoacetoxyethyl methacrylate, and then treated with 11 grams of triethylamine and 2.5 grams of initiator (AIBN). To this mixture was added 1000 ml deoxygenated water followed by 10 grams of ethylene diamine in 20 grams of water. The dispersion was heated to 65° C., held there with stirring for

2 hours and heated further to 80° C. for 10 hours. The resulting dispersion of the urethane acrylic copolymer had an acid number of 11.

P7 (Epoxy Dispersion)

An organic phase was made by dissolving 270 grams of Carboset® 525 acrylic copolymer (BF Goodrich Specialty Chemicals) followed by 630 grams of Epon® 1001F epoxy resin (Shell Chemical Co.), in 2100 grams of a 90:10 solvent mixture of ethyl acetate and acetone. 1000 grams of the organic phase was then neutralized with 40 grams of isopropanol and 19.5 grams of triethyl amine. An aqueous phase was prepared by mixing 220 grams of a 10% Alkanol® XC surfactant solution with 37 grams of a 30% poly(vinyl alcohol) solution (Aldrich, Cat. No. 36,062-7) and 1943 grams of water. The neutralized organic and aqueous phases were mixed and passed through a microfluidizer for 5 passes at 3500 psi. Volatile solvents were stripped from the dispersed mixture by purging the space above the dispersion with nitrogen at 35° C. or by removing with a rotary evaporator. The resulting dispersion was approximately 14% solids, and had a particle size of 100 nm and a Tg of 44° C.

P8 (Epoxy Dispersion)

This dispersion was made in a similar fashion to P7 but used 450 grams of Carboset® 525 and 450 grams of an epoxy resin sold by Aldrich Chemical Company under Catalog Number 40,804-2. The resulting dispersion had a particle size of 100 nm and a Tg of 38° C.

P9 (Polyester Ionomer Dispersion)

AQ-55, a polyester ionomer dispersion, was used as-received from Eastman Chemical Co. The Tg of this material was 55° C.

P10 (Polyurethane Dispersion)

The same preparation scheme was used as for P3 except bisphenol A was substituted for a portion of the 1,4-butanediol and the relative amounts of other components were adjusted such that the monomer feed ratio on a weight basis was 41.0% polycarbonate polyol, 3.9% dimethylol propionic acid, 8.1% butanediol, 6.2% bisphenol A and 40.0% isophorone diisocyanate. Tetrahydrofuran was removed by heating under vacuum to give an aqueous dispersion at 27.8% solids. Glass transition temperature was 42° C. as measured by DSC, and weight average molecular weight was 34,100.

P11 (Polyurethane Dispersion)

The same preparation scheme was used as for P5 except that the polycarbonate polyol content was reduced from 44% to 42% and the remaining 2% was replaced by an amino-propyl end-functionalized polysiloxane PS510, obtained from Petrarch. Tetrahydrofuran was removed by heating under vacuum to give an aqueous dispersion at 23.7% solids. Glass transition temperature was 30° C. as measured by DSC, and weight average molecular weight was 19,600.

P12 Polyethylene Dispersion

ChemCor® Emulsion 260, an anionic high density polyethylene emulsion, P12, was purchased from Chemical Corporation of America and used as received.

P13 Ethyl Acrylate/Vinylidene Chloride/Itaconic Acid Latex (10/88/2)

The same preparation was used as for the polymer P2 except itaconic acid was substituted for hydroxyethyl acrylate. The Tg of the polymer was 9° C. and the particle size was 77 nm.

P14 Acrylonitrile/Vinylidene Chloride/Acrylic Acid Latex (39/59/2)

The same preparation was used as for the polymer P2 except for using 59.67 g of acrylonitrile, 90.27 g of

vinylidene chloride and 3.06 g of acrylic acid. The Tg of the polymer is 79° C. and the particle size was 85 nm.

P15 Methyl Acrylate/Vinylidene Chloride/Itaconic Acid Latex (15/83/2)

The same preparation was used as for the polymer P2 except for using 22.95 g of methylacrylate, 126.99 g of vinylidene chloride and 3.06 g of itaconic acid. The Tg of the polymer is 25° C. and the particle size was 97 nm.

Additional Materials

(1) Airvol® 203 poly(vinyl alcohol) (PVA) was obtained from Air Products which was 87 to 89% hydrolyzed (by hydrolyzed is meant that the acetate groups in the monomeric units are converted to hydroxy groups) and had a number-average molecular weight of 12,000 and a weight-average molecular weight of 35,000.

(2) CX-100®, a polyfunctional aziridine crosslinker for the polyurethane-acrylic copolymer dispersion, was obtained from Neo Resins (a division of Avecia).

(3) Protex® 6L, a protease enzyme, was purchased from Genencor, liquid, used as received.

(4) Accusol® 882, a water-soluble associative thickener used as a viscosifying agent, was obtained from Rohm & Haas, Inc. and used as received.

(5) Poly(ethyl oxazoline) was purchased from Aldrich Chem. Co. and used as received.

Photographic Sample Preparation

Samples was prepared by coating in sequence blue-light sensitive layer, interlayer, green-light sensitive layer, UV layer, red-light sensitive layer, UV layer and overcoat on photographic paper support. The components in each individual layer are described below.

Blue Sensitive Emulsion (Blue EM-1): A high chloride silver halide emulsion is precipitated by adding approximately equimolar silver nitrate and sodium chloride solutions into a well stirred reactor containing glutaryl diaminophenyl disulfide, gelatin peptizer and thioether ripener. Cesium pentachloronitrosylsulfate(II) dopant is added during the silver halide grain formation for most of the precipitation, followed by the addition of potassium hexacyanoruthenate(II), potassium (5-methylthiazole)-pentachloroiodate, a small amount of KI solution, and shelling without any dopant. The resultant emulsion contains cubic shaped grains having edge length of 0.6  $\mu$ m. The emulsion is optimally sensitized by the addition of a colloidal suspension of aurous sulfide and heat ramped to 60° C. during which time blue sensitizing dye BSD-4, potassium hexachloroiodate, Lippmann bromide and 1-(3-acetamidophenyl)-5-mercaptopotetrazole were added.

Green Sensitive Emulsion (Green EM-1): A high chloride silver halide emulsion is precipitated by adding approximately equimolar silver nitrate and sodium chloride solutions into a well stirred reactor containing, gelatin peptizer and thioether ripener. Cesium pentachloronitrosylsulfate(II) dopant is added during the silver halide grain formation for most of the precipitation, followed by the addition of potassium (5-methylthiazole)-pentachloroiodate. The resultant emulsion contains cubic shaped grains of 0.3  $\mu$ m in edge length size. The emulsion is optimally sensitized by the addition of glutaryl diaminophenyl disulfide, a colloidal suspension of aurous sulfide and heat ramped to 55° C. during which time potassium hexachloroiodate doped Lippmann bromide, a liquid crystalline suspension of green sensitizing dye GSD- 1, and 1-(3-acetamidophenyl)-5-mercaptopotetrazole were added.

Red Sensitive Emulsion (Red EM-1): A high chloride silver halide emulsion is precipitated by adding approximately equimolar silver nitrate and sodium chloride solu-

tions into a well stirred reactor containing gelatin peptizer and thioether ripener. During the silver halide grain formation, potassium hexacyanoruthenate(II) and potassium (5-methylthiazole)-pentachloroiridate are added. The resultant emulsion contains cubic shaped grains of 0.4  $\mu\text{m}$  in edge length size. The emulsion is optimally sensitized by the addition of glutaryl diaminophenyl disulfide, sodium thiosulfate, tripotassium bis{2-[3-(2-sulfobenzamido) phenyl]-mercaptotetrazole} gold(I) and heat ramped to 64° C. during which time 1-(3-acetamidophenyl)-5- mercaptotetrazole, potassium hexachloroiridate, and potassium bromide are added. The emulsion is then cooled to 40° C., pH adjusted to 6.0 and red sensitizing dye RSD-1 is added.

Coupler dispersions were emulsified by methods well known in the art. The following imaging layers were coated in sequence on polyethylene-laminated photographic paper.

| Layer                                | Item                                                                       | Laydown (mg/ $\text{ft}^2$ ) |
|--------------------------------------|----------------------------------------------------------------------------|------------------------------|
| <u>Layer 1 Blue Sensitive Layer</u>  |                                                                            |                              |
|                                      | Gelatin                                                                    | 122.0                        |
|                                      | Blue sensitive silver (Blue EM-1)                                          | 22.29                        |
|                                      | Y-4                                                                        | 38.49                        |
|                                      | ST-23                                                                      | 44.98                        |
|                                      | Tributyl Citrate                                                           | 20.24                        |
|                                      | ST-24                                                                      | 11.25                        |
|                                      | ST-16                                                                      | 0.883                        |
|                                      | Sodium Phenylmercaptotetrazole                                             | 0.009                        |
|                                      | Piperidino hexose reductone                                                | 0.2229                       |
|                                      | 5-chloro-2-methyl-4-isothiazolin-3-one/2- methyl-4-isothiazolin-3-one(3/1) | 0.019                        |
|                                      | SF-1                                                                       | 3.40                         |
|                                      | Potassium chloride                                                         | 1.895                        |
|                                      | Dye-1                                                                      | 1.375                        |
| <u>Layer 2 Interlayer</u>            |                                                                            |                              |
|                                      | Gelatin                                                                    | 69.97                        |
|                                      | ST-4                                                                       | 9.996                        |
|                                      | Diundecyl phthalate                                                        | 18.29                        |
|                                      | 5-chloro-2-methyl-4-isothiazolin-3-one/2- methyl-4-isothiazolin-3-one(3/1) | 0.009                        |
|                                      | Catechol disulfonate                                                       | 3.001                        |
|                                      | SF-1                                                                       | 0.753                        |
| <u>Layer 3 Green Sensitive Layer</u> |                                                                            |                              |
|                                      | Gelatin                                                                    | 110.96                       |
|                                      | Green sensitive silver (Green EM-1)                                        | 9.392                        |
|                                      | M-4                                                                        | 19.29                        |
|                                      | Oleyl Alcohol                                                              | 20.20                        |
|                                      | Diundecyl phthalate                                                        | 10.40                        |
|                                      | ST-1                                                                       | 3.698                        |
|                                      | ST-3                                                                       | 26.39                        |
|                                      | Dye-2                                                                      | 0.678                        |
|                                      | 5-chloro-2-methyl-4-isothiazolin-3-one/2- methyl-4-isothiazolin-3-one(3/1) | 0.009                        |
|                                      | SF-1                                                                       | 2.192                        |
|                                      | Potassium chloride                                                         | 1.895                        |
|                                      | Sodium Phenylmercaptotetrazole                                             | 0.065                        |
| <u>Layer 4 M/C Interlayer</u>        |                                                                            |                              |
|                                      | Gelatin                                                                    | 69.97                        |
|                                      | ST-4                                                                       | 9.996                        |
|                                      | Diundecyl phthalate                                                        | 18.29                        |
|                                      | Acrylamide/t-Butylacrylamide sulfonate copolymer                           | 5.026                        |
|                                      | Bis-vinylsulfonylmethane                                                   | 12.91                        |
|                                      | 3,5-Dinitrobenzoic acid                                                    | 0.009                        |
|                                      | Citric acid                                                                | 0.065                        |
|                                      | Catechol disulfonate                                                       | 3.001                        |
|                                      | 5-chloro-2-methyl-4-isothiazolin-3-one/2- methyl-4-isothiazolin-3-one(3/1) | 0.009                        |

-continued

| Layer                              | Item                                                                                    | Laydown (mg/ $\text{ft}^2$ ) |
|------------------------------------|-----------------------------------------------------------------------------------------|------------------------------|
| <u>Layer 5 Red Sensitive Layer</u> |                                                                                         |                              |
| 10                                 | Gelatin                                                                                 | 125.96                       |
|                                    | Red Sensitive silver (Red EM-1)                                                         | 17.49                        |
|                                    | IC-35                                                                                   | 21.59                        |
|                                    | IC-36                                                                                   | 2.397                        |
|                                    | UV-1                                                                                    | 32.99                        |
|                                    | Dibutyl sebacate                                                                        | 40.49                        |
|                                    | Tris(2-ethylhexyl)phosphate                                                             | 13.50                        |
|                                    | Dye-3                                                                                   | 2.127                        |
|                                    | Potassium p-toluenethiosulfonate                                                        | 0.242                        |
|                                    | 5-chloro-2-methyl-4-isothiazolin-3-one/2- methyl-4-isothiazolin-3-one(3/1)              | 0.009                        |
|                                    | Sodium Phenylmercaptotetrazole                                                          | 0.046                        |
|                                    | SF-1                                                                                    | 4.868                        |
| 20                                 | <u>Layer 6 UV Overcoat</u>                                                              |                              |
|                                    | Gelatin                                                                                 | 76.47                        |
|                                    | UV-2                                                                                    | 3.298                        |
|                                    | UV-1                                                                                    | 18.896                       |
|                                    | ST-4                                                                                    | 6.085                        |
|                                    | SF-1                                                                                    | 1.162                        |
|                                    | Tris(2-ethylhexyl)phosphate                                                             | 7.404                        |
|                                    | 5-chloro-2-methyl-4-isothiazolin-3-one/2- methyl-4-isothiazolin-3-one(3/1)              | 0.009                        |
| 30                                 | <u>Layer 7 SOC</u>                                                                      |                              |
|                                    | Gelatin                                                                                 | 60.0                         |
|                                    | SF-1                                                                                    | 1.0                          |
|                                    | SF-2                                                                                    | 0.39                         |
| 40                                 | <chem>*c1cc2c(cc1[n+]3cc(*)c(*)cc3S(=O)(=O)C)S2</chem>                                  |                              |
| 45                                 | <chem>*c1cc2c(cc1[n+]3cc(*)c(*)cc3S(=O)(=O)C)C=CC=C2[n+]4cc(*)cc(*)cc4S(=O)(=O)C</chem> |                              |
| 50                                 | <chem>*c1cc2c(cc1[n+]3cc(*)c(*)cc3S(=O)(=O)C)C=CC=C2[n+]4cc(*)cc(*)cc4S(=O)(=O)C</chem> |                              |
| 55                                 | <chem>*c1cc2c(cc1[n+]3cc(*)c(*)cc3S(=O)(=O)C)C=CC=C2[n+]4cc(*)cc(*)cc4S(=O)(=O)C</chem> |                              |
| 60                                 | <chem>*c1cc2c(cc1[n+]3cc(*)c(*)cc3S(=O)(=O)C)C=CC=C2[n+]4cc(*)cc(*)cc4S(=O)(=O)C</chem> |                              |
| 65                                 | <chem>*c1cc2c(cc1[n+]3cc(*)c(*)cc3S(=O)(=O)C)C=CC=C2[n+]4cc(*)cc(*)cc4S(=O)(=O)C</chem> |                              |

-continued

| Layer | Item | Laydown (mg/ft <sup>2</sup> ) |
|-------|------|-------------------------------|
|       |      | 5                             |



M-4



IC-35



IC-36

Dye-1

-continued

| Layer | Item | Laydown (mg/ft <sup>2</sup> ) |
|-------|------|-------------------------------|
|       |      | 5                             |



Dye-2



Dye-3



ST-16

-continued

| Layer | Item                                                                               | Laydown (mg/ft <sup>2</sup> )                                                                                                                                                                                                                                                                                                                                                                                                                                                                                                                                                                                                                                                                               |                                              |
|-------|------------------------------------------------------------------------------------|-------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|----------------------------------------------|
| 5     |   |                                                                                                                                                                                                                                                                                                                                                                                                                                                                                                                                                                                                                                                                                                             |                                              |
| 10    | ST-23<br>+<br>ST-24                                                                |                                                                                                                                                                                                                                                                                                                                                                                                                                                                                                                                                                                                                            |                                              |
| 15    |  | All samples were exposed to $\frac{1}{10}$ seconds of daylight of color temperature 3000K, through 0-3 density step chart in combination with a heat-absorbing filter. After exposure, samples were processed (45 seconds) with the Kodak RA4 process to generate density and assess developability. Samples were also exposed to red, green and blue light and then RA-4 processed to generate cyan, magenta and yellow images. All samples having the overcoats of this invention produced satisfactory developed images as did the comparison samples without the overcoats of this invention.                                                                                                           |                                              |
| 20    |                                                                                    | Test for Water Resistance:                                                                                                                                                                                                                                                                                                                                                                                                                                                                                                                                                                                                                                                                                  |                                              |
| 25    |                                                                                    | Aqueous solutions of Ponceau Red dye are known to stain gelatin through ionic interaction and therefore are used to test water resistance of the overcoats. Ponceau Red dye solution was prepared by dissolving 1 gram dye in 1000 grams mixture of acetic acid and water (5 parts: 95 parts).                                                                                                                                                                                                                                                                                                                                                                                                              |                                              |
| 30    |                                                                                    | Samples, without being exposed to light, were processed through the Kodak RA4 process to obtain white Dmin samples. The water resistance test was done by placing a drop of the dye solution on the sample for 10 minutes followed by a 30-second water rinse to removed excess dye solution on the coating surface. Each sample was then air dried, and status A reflectance density on the spotted area was recorded. Assuming that the optical density of a Dmin check image with no protective overcoat corresponds to 0% water resistance and that an optical density of 0 corresponds to 100% water resistance, the percent water resistance for a sample is calculated using the following equation. |                                              |
| 35    |                                                                                    | Percent water resistance=100[1-(status A density of sample/status A density of check)]                                                                                                                                                                                                                                                                                                                                                                                                                                                                                                                                                                                                                      |                                              |
| 40    |                                                                                    | 45                                                                                                                                                                                                                                                                                                                                                                                                                                                                                                                                                                                                                                                                                                          |                                              |
| 45    |                                                                                    | Example 1                                                                                                                                                                                                                                                                                                                                                                                                                                                                                                                                                                                                                                                                                                   |                                              |
| 50    |                                                                                    | Color photographic paper samples were prepared by replacing the standard gelatin-containing overcoat with an overcoat consisting of poly(vinyl alcohol) (PVA) and polymer P6 as described in Table 1. In the case of sample 1-C, the inventive protective overcoat was coated over a paper structure previously coated with layers 1 through 6 as described above.                                                                                                                                                                                                                                                                                                                                          |                                              |
| 55    |                                                                                    | 55                                                                                                                                                                                                                                                                                                                                                                                                                                                                                                                                                                                                                                                                                                          |                                              |
| 60    |                                                                                    | TABLE 1                                                                                                                                                                                                                                                                                                                                                                                                                                                                                                                                                                                                                                                                                                     |                                              |
|       | Example ID                                                                         | Overcoat Composition (in mg/sq. ft.)                                                                                                                                                                                                                                                                                                                                                                                                                                                                                                                                                                                                                                                                        | % Water resistance after standard processing |
| 60    | 1-A                                                                                | 60 gelatin                                                                                                                                                                                                                                                                                                                                                                                                                                                                                                                                                                                                                                                                                                  | 0                                            |
|       | 1-B                                                                                | 175 P6                                                                                                                                                                                                                                                                                                                                                                                                                                                                                                                                                                                                                                                                                                      |                                              |
|       |                                                                                    | 61 PVA                                                                                                                                                                                                                                                                                                                                                                                                                                                                                                                                                                                                                                                                                                      | 76                                           |
|       |                                                                                    | 1.75 CX-100                                                                                                                                                                                                                                                                                                                                                                                                                                                                                                                                                                                                                                                                                                 |                                              |
| 65    | 1-C                                                                                | 175 P6                                                                                                                                                                                                                                                                                                                                                                                                                                                                                                                                                                                                                                                                                                      |                                              |
|       |                                                                                    | 61 PVA                                                                                                                                                                                                                                                                                                                                                                                                                                                                                                                                                                                                                                                                                                      | 96                                           |
|       |                                                                                    | 1.75 CX-100                                                                                                                                                                                                                                                                                                                                                                                                                                                                                                                                                                                                                                                                                                 |                                              |

|   | Solution/Step          | Time (seconds) | Temperature (° F.)                        |
|---|------------------------|----------------|-------------------------------------------|
| 5 | (1) Prime SP Developer | 45             | 100                                       |
|   | (2) Prime Bleach-Fix   | 45             | 86-97                                     |
|   | (3) Prime Stabiliser   | 90             | 86-99                                     |
|   | (4) Drying             | As needed      | Generally at least 140; not to exceed 205 |

## Testing Photographic Samples

## Test For Photographic Development

15 All samples were exposed to  $\frac{1}{10}$  seconds of daylight of color temperature 3000K, through 0-3 density step chart in combination with a heat-absorbing filter. After exposure, samples were processed (45 seconds) with the Kodak RA4 process to generate density and assess developability. Samples were also exposed to red, green and blue light and then RA-4 processed to generate cyan, magenta and yellow images. All samples having the overcoats of this invention produced satisfactory developed images as did the comparison samples without the overcoats of this invention.

20 Test for Water Resistance:

25 Aqueous solutions of Ponceau Red dye are known to stain gelatin through ionic interaction and therefore are used to test water resistance of the overcoats. Ponceau Red dye solution was prepared by dissolving 1 gram dye in 1000 grams mixture of acetic acid and water (5 parts: 95 parts).

30 Samples, without being exposed to light, were processed through the Kodak RA4 process to obtain white Dmin samples. The water resistance test was done by placing a drop of the dye solution on the sample for 10 minutes followed by a 30-second water rinse to removed excess dye solution on the coating surface. Each sample was then air dried, and status A reflectance density on the spotted area was recorded. Assuming that the optical density of a Dmin check image with no protective overcoat corresponds to 0% water resistance and that an optical density of 0 corresponds to 100% water resistance, the percent water resistance for a sample is calculated using the following equation.

35

$$\text{Percent water resistance}=100[1-(\text{status A density of sample}/\text{status A density of check})]$$

45

## Example 1

50 Color photographic paper samples were prepared by replacing the standard gelatin-containing overcoat with an overcoat consisting of poly(vinyl alcohol) (PVA) and polymer P6 as described in Table 1. In the case of sample 1-C, the inventive protective overcoat was coated over a paper structure previously coated with layers 1 through 6 as described above.

55

TABLE 1

| Example ID | Overcoat Composition (in mg/sq. ft.) | Note       | % Water resistance after standard processing |
|------------|--------------------------------------|------------|----------------------------------------------|
| 60         | 60 gelatin                           | Comparison | 0                                            |
|            | 175 P6                               |            |                                              |
|            | 61 PVA                               | Invention  | 76                                           |
|            | 1.75 CX-100                          |            |                                              |
| 65         | 175 P6                               |            |                                              |
|            | 61 PVA                               | Invention  | 96                                           |
|            | 1.75 CX-100                          |            |                                              |

It is evident from Table 1 that use of the inventive overcoat greatly improves the water resistance relative to a conventional gelatin overcoat.

To determine the amount of PVA washed out during RA 4 processing, multiple 1-C coatings in Example 1 were run through RA 4 process and the seasoned developer solution, bleach/fix solution and wash solution were analyzed by Size Exclusion Chromatography as follows. Aliquots of sample were dried first and then re-dissolved in dimethyl sulfoxide containing 0.01M lithium nitrate. Jordi Gel GBR mix-bed column was used for the analysis and the column was calibrated with narrow molecular weight distribution pullulan standards between molecular weight 5900 and 788000. The PVA peak in analyzed sample was confirmed by matching the same elution time with standard pure PVA peak under the same experimental condition. The results were summarized in TABLE 1A, showing the relative amount of PVA washed out during each step of RA 4 processing.

TABLE 1A

| Total percentage amount of PVA washed out versus PVA coated | percentage of PVA washed out into the developer from the total | Percentage of PVA washed out into the bleach/fix from the total | percentage of PVA washed out into the wash from the total |
|-------------------------------------------------------------|----------------------------------------------------------------|-----------------------------------------------------------------|-----------------------------------------------------------|
| 86%                                                         | 55%                                                            | Undetectable                                                    | 45%                                                       |

The results in TABLE 1A indicate that at least 86% of PVA coated in 1-C was washed out during RA 4 process and 55% of that was washed out into developer solution and 45% of that was in bleach/fix solution.

### Example 2

Color photographic paper samples were prepared by replacing the conventional gelatin-based overcoat with overcoats using polymer P3. For Example 2-D, the standard process was modified to include 0.20% of Protex® 6L enzyme in the wash tank of the process, in order to facilitate the washing out and removal of gelatin from the overcoat layer.

TABLE 2

| Example ID | Overcoat Comparison (in mg/sq. ft.) |            | % Water resistance after standard processing |
|------------|-------------------------------------|------------|----------------------------------------------|
| 2-A        | 60 gelatin                          | Comparison | 0                                            |
| 2-B        | 160 P3                              | Comparison | 0                                            |
|            | 40 gelatin                          |            |                                              |
| 2-C        | 160 P3                              | Invention  | 90                                           |
|            | 40 PVA                              |            |                                              |
| 2-D*       | 160 P3                              | Comparison | 96                                           |
| (Fused)    | 40 gelatin                          |            |                                              |

\*Sample 2-D represents sample 2-B, fused at 320° F. and 1 in/sec prior to water resistance testing.

The data of Table 2 demonstrate that the water resistance afforded by incorporation of the water-dispersible particles is greatly enhanced by coating them in a hydrophilic binder capable of washing out prior to processor drying, either in a water-soluble, non-crosslinked binder such as PVA (Example 2-C). Coating the water-dispersible particles in conventional, crosslinked gelatin (Example 2-B) afforded poor water resistance to the processed and dried image. Water resistance can be obtained by fusing overcoats based on water-dispersible particles in crosslinked gelatin, as exemplified by Example 2-D, but this requires the additional time-consuming, labor-intensive and potentially damaging step of fusing by contact heating. The overcoats of this

invention offer significant advantages by not requiring fusing to provide water resistance.

### Example 3

Color paper samples were prepared by coating water-dispersible polyurethane particles in non-crosslinked gelatin in two different ways:

Method 1: A solution of Protex® 6L enzyme was mixed into an overcoat coating solution, containing gelatin and polyurethane P4, just prior to the point of coating application, at a ratio of 1 part enzyme to 10 parts gelatin. Separate experiments confirmed that the time between mixing and drying of the coating was sufficiently long that the enzyme digested the gelatin in the overcoat layer sufficiently to render the gelatin non-crosslinkable.

Method 2: A solution of Protex® 6L enzyme was mixed into an aqueous solution of poly(vinyl pyrrolidone) (PVP) at a ratio of 1 part enzyme to 4 parts PVP. This solution was coated, as the uppermost layer at a laydown of 80 mg/sq ft of PVP, over a next-to-uppermost layer containing gelatin and polyurethane. Separate experiments confirmed that the time between coating application and drying of the coating was sufficiently long that the enzyme delivered in the uppermost layer digested the gelatin in the next-to-uppermost layer sufficiently to render the gelatin non-crosslinkable, and that the PVP readily dissolves and is removed in photographic processing.

TABLE 3

| Example ID | Overcoat Composition (in mg/sq. ft.) | Method of Enzyme Delivery | Note       | % Water resistance after standard processing |
|------------|--------------------------------------|---------------------------|------------|----------------------------------------------|
| 3-A        | 60 gelatin                           | None                      | Comparison | 0                                            |
| 3-B        | 160 P4                               | None                      | Comparison | 0                                            |
|            | 40 gelatin                           |                           |            |                                              |
| 3-C        | 160 P4                               | Method 1                  | Invention  | 17%                                          |
|            | 40 enzyme-digested gelatin           |                           |            |                                              |
| 3-D*       | 160 P4                               | Method 2                  | Invention  | 61%                                          |
|            | 40 enzyme-digested gelatin           |                           |            |                                              |

It is evident from Table 3 that enzyme-digested gelatin is a suitable non-crosslinked hydrophilic binder for the layers containing the water-dispersible polymers of this invention, such that upon processing the gelatin is washed out, allowing the water-dispersible polymers to form a water-resistant layer.

### Example 4

Color photographic paper samples were prepared by replacing the conventional gelatin-based overcoat with overcoats using polymer P1.

TABLE 4

| Example ID | Overcoat Comparison (in mg/sq. ft.) |            | % Water resistance after standard processing |
|------------|-------------------------------------|------------|----------------------------------------------|
| 4-A        | 60 gelatin                          | Comparison | 0                                            |
| 4-B        | 160 P1                              | Comparison | 1                                            |
|            | 50 gelatin                          |            |                                              |
| 4-C        | 160 P1                              | Invention  | 99                                           |
|            | 50 PVA                              |            |                                              |

The data of Table 4 demonstrate that the water resistance afforded by incorporation of the water-dispersible particles is greatly enhanced by coating them in a hydrophilic binder

capable of washing out prior to processor drying, for example using a water-soluble, non-crosslinked binder such as PVA. Coating the water-dispersible particles in conventional, crosslinked gelatin affords poor water resistance to the processed and dried image.

Example 5

Color photographic paper samples were prepared by replacing the conventional gelatin-based overcoat with overcoats using polymer P2.

TABLE 5

| Example ID | Overcoat Comparison (in mg/sq. ft.) | Note       | % Water resistance after standard processing |
|------------|-------------------------------------|------------|----------------------------------------------|
| 5-A        | 60 gelatin                          | Comparison | 0                                            |
| 5-B        | 160 P2                              | Comparison | 5                                            |
|            | 50 gelatin                          |            |                                              |
| 5-C        | 160 P2                              | Invention  | 95                                           |
|            | 50 PVA                              |            |                                              |

The data of Table 5 demonstrate that the water resistance afforded by incorporation of the water-dispersible particles is greatly enhanced by coating them in a hydrophilic binder capable of washing out prior to processor drying, in a water-soluble, non-crosslinked binder such as PVA. Coating the water-dispersible particles in conventional, crosslinked gelatin affords poor water resistance to the processed and dried image.

Example 6

Color photographic paper samples were prepared by replacing the standard gelatin-containing overcoat with an overcoat consisting of poly(vinyl alcohol) (PVA) and polymer P9. In the case of sample 6-C, the inventive protective overcoat was coated over a paper structure previously coated with layers 1 through 6 as described above.

TABLE 6

| Example ID | Overcoat Comparison (in mg/sq. ft.) | Note       | % Water resistance after standard processing |
|------------|-------------------------------------|------------|----------------------------------------------|
| 6-A        | 60 gelatin                          | Comparison | 0                                            |
| 6-B        | 175 P9                              | Invention  | 97                                           |
|            | 61 PVA                              |            |                                              |
| 6-C        | 175 P9                              | Invention  | >95                                          |
|            | 61 PVA                              |            |                                              |

It is evident from Table 6 that use of the inventive overcoat greatly improves the water resistance relative to a conventional gelatin overcoat.

Example 7

Color photographic paper samples were prepared by replacing the standard gelatin-containing overcoat with overcoats containing polymer P7.

TABLE 7

| Example ID | Overcoat Comparison (in mg/sq. ft.) | Note       | % Water resistance after standard processing |
|------------|-------------------------------------|------------|----------------------------------------------|
| 7-A        | 60 gelatin                          | Comparison | 0                                            |
| 7-B        | 140 P7                              | Comparison | 0                                            |
|            | 21 gelatin                          |            |                                              |

TABLE 7-continued

| Example ID | Overcoat Comparison (in mg/sq. ft.)              | Note      | % Water resistance after standard processing |
|------------|--------------------------------------------------|-----------|----------------------------------------------|
| 7-C        | 140 P7<br>55 PVA<br>15 Accusol® 882<br>thickener | Invention | 99                                           |

It is evident from Table 7 that use of the inventive overcoat greatly improves the water resistance relative to a conventional gelatin overcoat, and that the use of a water-soluble uncrosslinked hydrophilic binder such as PVA is advantaged over the use of crosslinked gelatin as a binder for the water-dispersible particles.

Example 8

Color photographic paper samples were prepared by replacing the standard gelatin-containing overcoat with overcoats containing polymer P8.

TABLE 8

| Example ID | Overcoat Comparison (in mg/sq. ft.) | Note       | % Water resistance after standard processing |
|------------|-------------------------------------|------------|----------------------------------------------|
| 8-A        | 60 gelatin                          | Comparison | 0                                            |
| 8-B        | 140 P8<br>45 PVA<br>13 Accusol® 882 | Invention  | 98                                           |

It is evident from Table 8 that use of the inventive overcoat greatly improves the water resistance relative to a conventional gelatin overcoat.

Example 9

Color photographic paper samples were prepared by replacing the standard gelatin-containing overcoat with overcoats containing polymers P5 or P10.

TABLE 9

| Example ID | Overcoat Comparison (in mg/sq. ft.) | Note       | % Water resistance after standard processing |
|------------|-------------------------------------|------------|----------------------------------------------|
| 9-A        | 60 gelatin                          | Comparison | 0                                            |
| 9-B        | 160 P5                              | Comparison | 0                                            |
|            | 50 gelatin                          |            |                                              |
| 9-C        | 160 P10                             | Comparison | 0                                            |
|            | 50 gelatin                          |            |                                              |
| 9-D        | 160 P5<br>50 PVA                    | Invention  | >99                                          |
| 9-E        | 160 P10<br>50 PVA                   | Invention  | >99                                          |

It is evident from Table 9 that use of the inventive overcoat greatly improves the water resistance relative to a conventional gelatin overcoat, and that the use of a water-soluble uncrosslinked hydrophilic binder such as PVA is advantaged over the use of crosslinked gelatin as a binder for the water-dispersible particles.

Example 10

Color photographic paper samples were prepared by replacing the standard gelatin-containing overcoat with overcoats containing polymer P11.

TABLE 10

| Example ID | Overcoat Comparison (in mg/sq. ft.) | Note       | % Water resistance after standard processing |
|------------|-------------------------------------|------------|----------------------------------------------|
| 10-A       | 60 gelatin                          | Comparison | 0                                            |
| 10-B       | 160 P11<br>50 PVA                   | Invention  | >99                                          |

It is evident from Table 10 that use of the inventive overcoat greatly improves the water resistance relative to a conventional gelatin overcoat.

#### Example 11

Color photographic paper samples were prepared by replacing the standard gelatin-containing overcoat with an overcoat consisting of poly(vinyl alcohol) (PVA) or poly(ethyl oxazoline) (PEOX) and polymer P12-P15 as described in Table 11. In the case of example 16, the inventive protective overcoat was coated over a paper structure previously coated with layers 1 through 6 as described above.

TABLE 11

| Example ID | Overcoat Comparison (in mg/sq. ft.) | Note       | % Water resistance after standard processing |
|------------|-------------------------------------|------------|----------------------------------------------|
| 11A        | 60 gelatin                          | Comparison | 0                                            |
| 11B        | 175 P12<br>61 PVA                   | Invention  | 89                                           |
| 11C        | 175 P13<br>61 PVA                   | Invention  | 97                                           |
| 11D        | 175 P14<br>61 PVA<br>1.75 CX 100    | Invention  | 86                                           |
| 11E        | 175 P15<br>61 PVA<br>1.75 CX 100    | Invention  | 93                                           |
| 11F        | 175 P13<br>44 PEOx                  | Invention  | 97                                           |

It is evident from Table 11 that use of the inventive overcoats greatly improves the water resistance relative to a conventional gelatin overcoat.

The invention has been described in detail with particular reference to certain preferred embodiments thereof, but it will be understood that variations and modifications can be effected within the spirit and scope of the invention.

What is claimed is:

1. A photographic element comprising:
  - (a) a support;
  - (b) at least one silver-halide emulsion layer superposed on a side of said support; and
  - (c) overlying the silver emulsion layer, a processing-solution-permeable protective overcoat having a lay-down of at least 0.54 g/m<sup>2</sup> (50 mg/ft<sup>2</sup>) made from a coating composition comprising the following:
    - (i) 30 to 95%, by weight of solids, of water-dispersible polymer in the form of particles having an average particle size of less than 500 nm and a T<sub>g</sub> between -40° C. and 80° C., and
    - (ii) 5 to 70%, by weight of solids, of water-soluble polymer such that more than 30 weight percent of water-soluble polymer is washed out during photographic processing,

wherein the composition is essentially free of polyurethane and polyester polymer, wherein the weight ratio of the

water-dispersible polymer to the water-soluble polymer is between 50:50 to 90:10, wherein the applied overcoat comprises less than 5% by weight of gelatin, and whereby the overcoat forms a water-resistant overcoat after photoprocessing.

5 2. The photographic element of claim 1 wherein said water-dispersible polymer is selected from the group consisting of polyamides, polyureas, polyethers, polycarbonates, polyacid anhydrides, and polymers comprising combinations thereof; and polymers derived from vinyl ethers, vinyl heterocyclic compounds, styrenes, olefins, halogenated olefins, unsaturated acids and esters thereof, unsaturated nitrites, vinyl alcohols, acrylamides and methacrylamides, and vinyl ketones, and copolymers formed from various combinations of the corresponding monomers, and combinations thereof.

10 3. The imaging photographic element of claim 2 wherein said water-dispersible polymer comprises ionized or ionizable groups.

15 4. The imaging photographic element of claim 1 wherein said water-soluble polymer is selected from the group consisting of polyvinyl alcohol, cellulose ethers, poly(N-vinyl amides), polyacrylamides, polyesters, poly(ethylene oxide), dextrans, starch, noncrosslinked gelatin, whey, albumin, poly(acrylic acid), poly(ethyl oxazolines), alginates, gums, poly(methacrylic acid), poly(oxymethylene), poly(ethyleneimine), poly(ethylene glycol methacrylate), poly(hydroxy-ethyl methacrylate), poly(vinyl methyl ether), poly(styrene sulfonic acid), poly(ethylene sulfonic acid), poly(vinyl phosphoric acid) and poly(maleic acid), and combinations thereof.

20 5. The imaging photographic element of claim 1 wherein the weight average molecular weight of said water soluble polymer is less than or equal to 300,000.

25 6. The composition of claim 1 wherein the weight average molecular weight of said water-soluble polymer is 1500 to 100,000.

30 7. The composition of claim 6 wherein said water-soluble polymer is polyvinyl alcohol having a weight average molecular weight of less than or equal to about 100,000, with the proviso that if said molecular weight is greater than about 70,000, then the degree of hydrolysis is less than 95%.

35 8. The photographic element of claim 1 wherein the support comprises polymeric films, papers or glass.

40 9. The photographic element of claim 1 wherein the overcoat composition further comprises UV absorbers, surfactants, emulsifiers, coating aids, lubricants, matte particles, rheology modifiers, crosslinking agents, antifoggants, inorganic fillers, pigments, magnetic particles and/or biocides.

45 10. A method of making a photographic print comprising:

- (a) providing a photographic element comprising a support, a silver-halide emulsion layer superposed on a side of said support, a processing-solution-permeable coating overlying the silver-halide emulsion layer, said protective overcoat comprising having a lay-down of at least 0.54 g/m<sup>2</sup> (50 mg/ft<sup>2</sup>) made from a coating composition 30 to 95%, by weight of solids, of water-dispersible polymer in the form of particles having an average particle size of less than 500 nm and a T<sub>g</sub> between -40° C. and 80° C., and 5 to 70%, by weight of solids, of water-soluble polymer such that more than 30 weight percent of the water-soluble polymer is washed out during photographic processing wherein the weight ratio of water-dispersible polymer to water-soluble polymer in the coating composition is between 50:50 to 90:10 and comprising less than 5% by weight

**37**

of gelatin in the applied overcoat, which said overcoat is essentially free of water-dispersible polyurethane or polyester,

(b) developing the photographic element in a developer solution having a pH greater than 7 to obtain the photographic print; and

(c) drying the photographic element to a temperature under 60° C. to render the overcoat water-resistant in the final product.

**11.** The method of claim **10** wherein said water-dispersible polymer is selected from the group consisting of polyamides, polyureas, polyethers, polycarbonates, polyacid anhydrides, and polymers comprising combinations thereof; and polymers derived from vinyl ethers, vinyl heterocyclic compounds, styrenes, olefins, halogenated olefins, unsaturated acids and esters thereof, unsaturated nitriles, vinyl alcohols, acrylamides and methacrylamides, and vinyl ketones, and copolymers thereof, and combinations thereof.

**12.** The method of claim **11** wherein said water-dispersible polymer comprises ionized or ionizable groups.

**38**

**13.** The method of claim **10** wherein said water-soluble polymer is selected from the group consisting of polyvinyl alcohol, cellulose ethers, poly(N-vinyl amides), polyacrylamides, polyesters, poly(ethylene oxide), dextrans, starch, uncrosslinked gelatin, whey, albumin, poly(acrylic acid), poly(ethyl oxazolines), alginates, gums, poly(methacrylic acid), poly(oxymethylene), poly(ethyleneimine), poly(ethylene glycol methacrylate), poly(hydroxy-ethyl methacrylate), poly(vinyl methyl ether), poly(styrene sulfonic acid), poly(ethylene sulfonic acid), poly(vinyl phosphoric acid) and poly(maleic acid), and combinations thereof.

**14.** The method of claim **10** wherein the weight average molecular weight of said water soluble polymer is less than 300,000.

**15.** The method of claim **10** wherein the weight average molecular weight of said water-soluble polymer is 1500 to 100,000.

\* \* \* \* \*